

1

3,523,750

## PROCESS FOR TREATMENT OF PROTEINACEOUS MATERIALS

Giuliana C. Tesoro, Dobbs Ferry, N.Y., assignor to J. P. Stevens & Co., Inc., New York, N.Y., a corporation of Delaware  
No Drawing. Continuation-in-part of application Ser. No. 569,016, Aug. 1, 1966, which is a continuation-in-part of application Ser. No. 481,094, Aug. 19, 1965. This application Nov. 8, 1968, Ser. No. 774,508  
Int. Cl. D06n 13/48

U.S. Cl. 8—127.6

26 Claims

### ABSTRACT OF THE DISCLOSURE

This invention concerns a novel process for modifying proteinaceous substrates comprising treating said substrates with polyfunctional aziridine reagent, and heating the treated substrate until the desired modification takes place.

The present invention is a continuation-in-part of my copending application Ser. No. 569,016, filed Aug. 1, 1966 now abandoned, which is a continuation-in-part of my application Ser. No. 481,094, filed Aug. 19, 1965, now abandoned.

The present invention relates to novel processes for treatment of proteinaceous materials and more particularly processes for enhancing the properties and characteristics of textiles containing wool fibers and improved products obtained thereby.

Various methods have been devised for the treatment of textile fabrics containing wool in order to improve certain properties thereof. Particularly important to the wool industry are methods and compositions to bring about improvements in the dimensional stability and the felting characteristics of textiles containing wool fibers. Although many methods have been developed for wool treatment, relatively few give satisfactory results from the standpoint of improvement in dimensional stability and felting. Moreover, prior known methods frequently may deleteriously and adversely affect the appearance, handle, strength and other properties of the woolen textiles.

Accordingly, it is the object of the present invention to provide novel processes for imparting improved properties to proteinaceous materials, particularly wool-containing textile materials, which overcome the shortcomings and disadvantages associated with prior methods and compositions.

It is a further object of the present invention to provide novel processes for imparting excellent properties and characteristics to wool-containing textiles which avoid the drawbacks of prior methods and compositions.

It is a further object of the present invention to provide novel processes for imparting to wool-containing textile material excellent properties of dimensional stability and resistance to felting.

It is a further object of the present invention to provide woolen textiles having improved properties, particularly dimensional stability.

It is a further object of the present invention to provide processes for treating wool-containing textile materials without adversely affecting the appearance, handle, strength and other desirable properties of the textile.

It is a further object of the present invention to pro-

2

vide processes for treating wool-containing fabrics which have desirable surface appearance after laundering, particularly minimal fuzziness.

In attaining the above objects, one feature of the present invention resides in imparting excellent properties and characteristics to proteinaceous materials by treating textile materials containing wool fibers with a selected group of polyfunctional compounds of a specified structure whereby the improvements in dimensional stability and other physical properties are achieved without adversely affecting the appearance, hand, strength and other desirable properties of the textile.

More particularly, a proteinaceous textile substrate such as wool and its blends is treated with a solution of polyfunctional composition represented by the structural formula:



20 wherein

A is selected from the group consisting of Az,



25 a is an integer from 1 to 4,

m is an integer from 2 to 4,

Az is



where

30 R<sup>1</sup>, R<sup>2</sup>, R<sup>3</sup> are selected from the group consisting of H and alkyl having from 1 to 4 carbon atoms,

35 J which has the valence of m is the residue of a polyol having at least 2 to 8 hydroxyl groups, after 2 to 4 hydroxyl groups have been removed, and

Q is selected from the group consisting of divalent aromatic and alkyl-substituted aromatic groups having 6 to 40 18 carbon atoms,

to deposit an amount sufficient to obtain the enhancement of properties sought, dried and cured at elevated temperatures until the properties of the substrate are enhanced.

45 While all of the above polyfunctional compositions function effectively as modifiers and enhancers of proteinaceous substrates, as in any large group, some members of the group, for various reasons, function more effectively than the others and for this reason are preferred. Thus, in the instant case, a more restricted group of compositions included within the above broad group, comprise the preferred compositions of this invention. These compositions are included within the structural formula:

Formula (I)



55 wherein

m is a number from 2 to 4,

Az is



60 65 R<sup>1</sup> and R<sup>2</sup>, are independently selected from the group consisting of H and alkyl having from 1 to 4 carbon atoms,

J which has the valence of *m* is the residue of an aliphatic or alicyclic polyol having from 2 to 4 hydroxyl groups after 2 to 4 hydroxyl groups have been removed, and Q is methylphenylene.

In the preferred process embodiment a woolen or wool blend substrate is contacted with an amount of one or more of the preferred treating agents, in the form of a liquid solution, sufficient to deposit a modifying or enhancing amount of agent and cured until the desired enhancement of properties is obtained. Ordinarily the concentration of treating agent required varies between about 0.25 to 10% by weight with the true upper limit determined primarily by economics. The mode of application is not critical; padding, spraying, dipping or the like being applicable. Depending upon the initial concentration of agent utilized, the pickup varies between about 50% to about 300%. Normally the treated substrate is dried and cured at about 100° C. to 200° C. for about 3 to 6 minutes, longer times being acceptable.

A further feature of the present invention resides in treating wool-containing textile materials with a group of polyaziridinyl compounds and with selected co-reactants in order to further enhance and improve the dimensional stability and other physical properties of the textile without adversely affecting the appearance, hand, strength and other desirable properties thereof.

A more specific feature of the present invention resides in treating wool-containing textile materials according to a process hereinafter defined with a certain group of relatively high molecular weight polyaziridinyl compounds in the presence of selected polybasic acids of polyamino compounds whereby excellent properties are imparted to the textile.

The above, as well as other objects, features and advantages of the present invention will become apparent from the following detailed description thereof.

According to the present invention, novel processes are provided whereby wool-containing textile materials, particularly woven and knitted fabrics containing wool fibers, are treated with selected polyfunctional compounds to impart dimensional stability and other desirable properties to the textile product without substantially adversely affecting the appearance, handle, strength and other mechanical properties thereof.

It has been observed that the dimension properties of wool-containing textile materials are considerably enhanced as a result of the novel processes of the present invention and further that the desired properties are obtained without causing undesirable discoloration, harshening or other undesirable side effects. Moreover, in accordance with a further aspect of the present invention, novel processes are provided whereby an enhancement in the physical properties of wool-containing textile materials, particularly dimensional stability, are obtained when the above-defined aziridine compounds are used in conjunction with co-reactants to be defined hereinafter which bring about an even greater improvement than was heretofore possible.

A detailed description of the substituents included within the formulae defining the polyfunctional compounds of this invention follows:

The compounds that are preferred for the present invention are polyfunctional compounds defined by Formula I, supra.

Aziridinyl compounds as defined by the symbol "Az" in the various formulas which are suitable for purposes of the present invention may be obtained by several means such as, for example, the methods disclosed in British Pat. No. 919,861, the entire disclosure of which is relied on and incorporated herein by reference. Briefly described, the aziridinyl compounds defined by Formula I, supra, may be prepared by reacting an organic polysiocyanate with, preferably, an organic compound containing at least two hydroxyl groups to produce an intermediate

having at least two isocyanate groups. Then the intermediate compound is reacted with a 1,2-alkylenimine to obtain the desired product. It has been determined that compounds falling within the scope of the Formula I, supra are exceptionally suitable for the treatment of wool-containing textile materials. It will be apparent from a consideration of the compounds encompassed by the present invention that the average molecular weight of the preferred compounds will range from about 1000 to about 6000. Such compounds are commercially available or can be prepared by known methods from commercially available raw materials.

#### GROUPS REPRESENTATIVE OF Q

|    | Name:                                                          | Composition                                                                       |
|----|----------------------------------------------------------------|-----------------------------------------------------------------------------------|
| 15 | Phenylene (o, m, or p)                                         | —C <sub>6</sub> H <sub>4</sub> —                                                  |
|    | Methylphenylene (various isomers such as 4-methyl-m-phenylene) | —C <sub>6</sub> H <sub>3</sub> (—CH <sub>3</sub> )—                               |
| 20 | (o, m, or p)-Phenylene-dimethylene                             | —H <sub>2</sub> CC <sub>6</sub> H <sub>4</sub> CH <sub>2</sub> —                  |
|    | Biphenylene                                                    | —C <sub>6</sub> H <sub>4</sub> C <sub>6</sub> H <sub>4</sub> —                    |
| 25 | Methylenedi-(o, m, or p)-phenylene                             | —C <sub>6</sub> H <sub>4</sub> CH <sub>2</sub> C <sub>6</sub> H <sub>4</sub> —    |
|    | Benzylphenylene                                                | —C <sub>6</sub> H <sub>3</sub> (—CH <sub>2</sub> C <sub>6</sub> H <sub>5</sub> )— |
|    | Naphthylene                                                    | —C <sub>10</sub> H <sub>6</sub> —                                                 |

The residue J can be (a) divalent, (b) trivalent, or (c) tetravalent.

(a) Illustrative of the residue J in the form of a divalent radical are the following:

- (II) (—CH<sub>2</sub>—)<sub>x</sub>, where *x* is a number from 1 to 100.  
 (III) (—C<sub>a</sub>H<sub>2a</sub>O—)<sub>x</sub>C<sub>a</sub>H<sub>2a</sub>, where *a* is a number from 1 to 4, and *x* is a number from about 1 to about 100, preferably from about 5 to about 40.  
 (IV) (—CH<sub>2</sub>CH=CHCH<sub>2</sub>—)<sub>u</sub>, which is derived from polybutadiene, wherein the average degree of polymerization, *u* is between about 6 and about 100.



which is one kind of linear polyester radical, where *n* is 2 to 6, and the average value of *v* is between about 3 and about 80.

- (VI) 
$$[(-\text{CH}_2-)_n-\text{O}-\text{C}(-\text{CH}_2-)_q-\text{C}-\text{O}]_r(-\text{CH}_2-)_n$$
- 50 which is another kind of linear polyester radical, where *n* is 2 to 6, *q* is 3 to 5, and *r* is 2 to 35.



55 where *a* is 1 to 4; *x* and *y* independently are 1 to 100; and *L* is a divalent alicyclic radical of 3 to 20 carbon atoms, C<sub>2</sub> to C<sub>20</sub> alkylene, or C<sub>2</sub> to C<sub>20</sub> alkylene having the chain interrupted by one to ten



groups in which *R* is H or alkyl having 1 to 5 carbon atoms.

60 In the general formula: J is derived from a polyol J(—OH)<sub>m</sub> having a molecular weight between about 500 and about 5,500.

65 For instance, suitable divalent radicals of the type represented for Formula VII are provided by condensation products of the alkoxylate type which can be formed from any of the following starting compounds HO—L—OH, which are given by way of example, by

- (A) Ethoxylation with approximately 10 to 125 mole-  
 70 parts of ethylene oxide,



In carrying out the present invention, the wool-containing textile material which may be in any suitable form such as fiber, yarn or fabric may be treated with the polyfunctional compounds defined by Formula I, generally by impregnation with a solution thereof.

The solvent vehicle may be aqueous or non-aqueous. The treating mixture of solvent and polyfunctional compound may be in the form of a solution, suspension, emulsion or the like. The textile material may be sprayed, padded, immersed, dipped, brushed or similarly contacted with the polyfunctional compound, thereafter dried and cured. Exposure to elevated temperature may be used to insolubilize the polyfunctional compound. Alternatively, the textile, after being contacted with the polyfunctional compound may be permitted to stand for a brief period so as to achieve insolubilization.

If desired, the treated wool-containing textile material may thereafter be washed to remove residual soluble chemicals which may interfere or adversely affect the properties of the final product. Excellent dimensional stability is imparted to woolen textiles treated in the aforementioned manner. When laundered by conventional procedures commonly used for cotton or hydrophobic fibers, the woolen textile materials treated in accordance with the present invention as well as garments made from such woolen textile materials do not exhibit noticeable felting, fuzzy appearance, shrinkage or other undesirable properties which would deleteriously affect the final quality of the garment.

The present invention constitutes a considerable advance over what has gone heretofore inasmuch as the treatment with the selected polyfunctional compounds does not deleteriously alter the color, hand or other aesthetic properties of the woolen textile and, moreover, does not substantially adversely impair the tensile strength, tear strength, abrasion resistance and other important properties of the textile material.

In accordance with a further preferred aspect of the present invention, textile materials containing wool are treated with the aziridine compounds represented by the Formula I supra in combination with the coreactants as defined hereinafter to achieve even greater enhancement of the dimensional stability and other desirable properties of the textile products. Suitable coreactants are polybasic acids and polyamine compounds particularly saturated aliphatic dicarboxylic acids containing from 2 to 12 carbon atoms and polyalkylene polyamines containing, for example, from 4 to 20 carbon atoms and 2 to 5 nitrogen atoms. Representative examples of acids include succinic acid, adipic acid, sebatic acid, citric acid, tartaric acid, polyacrylic acid, and the like. Examples of polyamines include diethylenetriamine, tetraethylenepentamine, hydroxyethylmethylenediamine, polyethyleneimines of wide molecular weight range, 1,3-diaminopropane, 1,6-diaminohexane, and the like.

In general, it has been observed that the coreactants will accelerate insolubilization of the polyfunctional compound in or on wool and will drive the polymerization reaction to completion in a shorter period of time. In addition, it has been observed that in certain respects the resulting properties of the textile are superior to that treated with the polyfunctional compound alone. It is, however,

15 to be noted that the invention does not require the presence of co-reactants in order to achieve satisfactory dimensional stability or other desirable properties in the wool-containing textile.

The treating mixture containing the polyfunctional compounds as defined by the structural Formula I and a vehicle therefor may take the form of a solution in organic solvents or water when feasible. The compounds may also be applied from aqueous emulsion which can be rapidly prepared by suitable choice of solvents and emulsifying agents. Because of their stability at room temperature over relatively long periods of time, solutions and emulsions of the treating agents of the present invention may normally be stored without special precautions being necessary.

30 According to a further more detailed aspect of the present invention, the wool-containing textile material may be treated with the above-defined polyfunctional compounds, either before or after dyeing because the treatment with aziridines does not alter or deleteriously affect the dyeing properties of the woolen textiles. No adverse effects on the rate and evenness of the dyeing have been observed, even if the treatment with the polyfunctional compound is carried out before the dyeing operation. Moreover, there is no change of shade or adverse effect on color-fastness if the treatment with the polyfunctional compound is applied to the textile after the dyeing operation. This aspect of the invention is particularly important from a commercial standpoint inasmuch as it allows a wider range of operating conditions and greater flexibility in carrying out the modification of the woolen textile product.

45 When carrying out the process of the invention utilizing arizidinyl compounds in combination with selected co-reactants as defined above, the treatment may be carried out in a single step or in several separate steps. Because of their nature, it is possible to use the polyfunctional 50 compounds as defined herein in a single step in conjunction with other functional finishes such as water and stain repellents, soil release agents and the like. The latter include the acrylics and their salts as well as the fluorocarbons. The ease of formulation and application of the 55 polyfunctional compounds makes them particularly suitable for use in combination with other finishes to impart permanent creasing properties to woolen fabrics.

No special precautions need be taken when carrying out the process of the present invention inasmuch as 60 the insolubilization reaction of the polyfunctional compound on the wool textile can take place at moderate temperatures. It is therefore possible to obtain the desired insolubilization reaction even by tumble-drying procedures which are especially desirable when the objective 65 is the stabilization of manufactured woven or knitted garments which cannot be conveniently processed in curing ovens at elevated temperature. Thus, the present invention provides a commercially feasible means for applying shrinkproofing finishes to manufactured garments in a convenient or simple method without requiring the use of complex equipment and procedures.

Applicable to wool textile materials in any form or shape, the present invention may be used to impart dimensional stability and other desired properties to wool fibers, 75 woolen and worsted yarn, woven or knitted fabrics and

- (B) Propoxylation with approximately 8 to 95 mole-parts of propylene oxide, or
- (C) Alkoxylation with a proportionate mole ratio of higher or mixed alkylene oxides.

## STARTING COMPOUNDS HO-L-OH PRIOR TO ALKOXYLATION

|                                |                                                                                                                                                                                                                           |
|--------------------------------|---------------------------------------------------------------------------------------------------------------------------------------------------------------------------------------------------------------------------|
| Ethylene glycol.....           | HO-CH <sub>2</sub> CH <sub>2</sub> -OH                                                                                                                                                                                    |
| Propylene glycol.....          | HO-CH(CH <sub>3</sub> )CH <sub>2</sub> -OH                                                                                                                                                                                |
| Trimethylene glycol.....       | HO-CH <sub>2</sub> CH <sub>2</sub> CH <sub>2</sub> -OH                                                                                                                                                                    |
| Decamethylene glycol.....      | HO-(CH <sub>2</sub> ) <sub>9</sub> -OH                                                                                                                                                                                    |
| Diethylene glycol.....         | HO-CH <sub>2</sub> CH <sub>2</sub> OCH <sub>2</sub> CH <sub>2</sub> -OH                                                                                                                                                   |
| 2-butene-1,4-diol.....         | HO-CH <sub>2</sub> CH=CHCH <sub>2</sub> OH                                                                                                                                                                                |
| 1,4-cyclohexanedimethanol..... | $  \begin{array}{c}  \text{CH}_2\text{CH}_2 \\    \qquad \quad \diagdown \\  \text{HO}-\text{CH}_2\text{CH} \qquad \text{CH}_2\text{CH}_2-\text{OH} \\    \qquad \quad \diagup \\  \text{CH}_2\text{CH}_2  \end{array}  $ |
| 2,2'-thiodiethanol.....        | HO-CH <sub>2</sub> CH <sub>2</sub> SCH <sub>2</sub> CH <sub>2</sub> -OH                                                                                                                                                   |
| Diethanolamines.....           | (HO-CH <sub>2</sub> CH <sub>2</sub> -) <sub>2</sub> N-R, wherein R is<br>alkyl having 1 to 5 carbon atoms, and<br>L is -CH <sub>2</sub> CH <sub>2</sub> N(R)CH <sub>2</sub> CH <sub>2</sub> -.                            |

When *trivalent*, the residue J is the radical remaining upon removal of 3 hydroxyls from a polyol higher in degree than a diol. Examples of the residue J in the trivalent form are represented by the individual compounds embraced within the following collective Formula VIII:



after removal of the 3 terminal hydrogen atoms, wherein the value of  $a$  is 1 to 4, while  $x$ ,  $y$ , and  $z$ , each ranging from 1 to about 100, denote mole-parts of one or more kinds of alkylene oxide  $C_aH_{2a}O$  condensed with a trihy-

6

dric starting compound,  $(HO)_3M$ , M being a trivalent organic radical. For instance, a suitable trivalent radical of the type represented by Formula VIII is derived from glycerol condensed with approximately 50 mole-parts of propylene oxide. In that case (referring to Formula VIII)

## 5 M is the radical



10 and  $a$  is 3, while the sum of  $x$ ,  $y$ , and  $z$  is 50. Other aliphatic starting compounds of the type  $(HO)_3M$  which may be alkylated (as by  $CH_2CH_2O$ ,  $C_3H_6O$ , and  $C_4H_8O$ ) are, for example, 2-methyl-1,2,3-propanetriol, butanetriols, hexanetriols, 2-alkyl-2-(hydroxymethyl)-1,3-propanediols (especially wherein the alkyl group has 3 or less carbon atoms), triethanolamine, and 2-dimethylamino)-2-(hydroxymethyl)-1,3 propanediol.

The m-valent residue J of the formulae is also provided by the condensation products which are alkylene oxide derivatives of many starting compounds other than those specifically named, whether the prealkoxylated compound is of the dihydric type  $\text{HO}-\text{L}-\text{OH}$  or of the trihydric type  $(\text{HO})_3\text{M}$ . Further examples of suitable starting compounds conforming to the types of  $\text{HO}-\text{L}-\text{OH}$  and  $(\text{HO})_3\text{M}$  will be found in British Pat. No. 919,861.

Typical of the methods whereby the aziridinyl compounds may be made is the procedure shown in Example XXVI which describes the reaction of a polyol and an isocyanate and the subsequent reaction with the alkyl-enimine.

Illustrative of the above compounds are:



garments. In general, for optimum effects to be realized, the fabric customarily contains appreciable proportion of wool fiber, generally 30% or more, 60 to 100% being the preferred range.

It will be apparent from the foregoing that the wool present in the textile can be by itself or present in a blend or admixture with other natural fibers such as cotton or with synthetic fibers such as polyamides, polyesters, polyolefins and acrylic fibers. The examples which appear hereinafter generally show the reaction condition suitable for obtaining satisfactory results. It will be noted, however, that the optimum conditions for processing any given fiber blend or mixture will be determined by many factors such as concentration of reagent, time of impregnation, temperature, atmospheric conditions, configuration, as well as other parameters. Conditions within the ranges discussed hereinafter will generally give satisfactory results on the textile materials indicated although these ranges are not to be construed as limiting the invention in any way.

For most purposes, the polyfunctional compounds employed in this invention are used in amount sufficient to keep shrinkage below 6% based upon the original dimensions of the substrate. Generally, between about 0.5 and 10% by weight add-on based upon the weight of the dry substrate is sufficient to keep shrinkage below the desired level. This add-on is referred to as a modifying amount of polyfunctional composition throughout this application. For example, in a typical embodiment where a 100% wool substrate is treated, add-on amounts of about 2% to about 5% based on the weight of the wool treated are preferred, although amounts outside these ranges may be used.

In accordance with the aspect of this invention relating to the combination of the aziridine compound and co-reactant, when the co-reactant is used, the amount thereof employed should be sufficient to provide approximately 0.5 to about 2.0 reactive groups of the co-reactant which is in the form of amino groups or carboxyl groups for each aziridinyl group of the aziridinyl compound defined by Formula I. In other words, approximately 0.5 to about 2.0 equivalents of the co-reactant, polyamine or polycarboxylic acid, should be present for each aziridinyl equivalent present. It has been determined that the co-reactant may be added to the treating solution which contains the aziridinyl compound of Formula I or can be applied in a separate step either before or after application of the aziridinyl compound. Properties and characteristics may vary somewhat depending upon the sequence of reaction; however, it has been observed that generally the order of reactants can be varied with equally satisfactory results.

As mentioned above, the aziridinyl compound can be applied to the wool-containing textile material in any convenient manner. Generally, the aziridinyl compound is dissolved at the desired concentration in an anhydrous organic solvent such as a hydrocarbon including toluene, xylene, petroleum fractions and similar materials, halogenated solvent such as carbon tetrachloride and perchloroethylene or any other convenient inert solvent in which the aziridinyl compound is soluble and which in itself will not adversely affect the woolen textile material or deleteriously interfere with the insolubilization of the aziridinyl compound or interfere with the functioning of the co-reactant if any is used.

The aziridinyl compound may be applied to the woolen textile substrate in the form of a self-emulsifiable concentrate which is diluted with water to the desired concentration prior to using same. In any event, the co-reactant polyamine or polycarboxylic acid may be added to the treating solution or emulsion containing the aziridinyl compound or the co-reactant may be applied in a separate step from a solution prepared from the same solvent as that used in connection with the aziridine compound, or a different organic solvent or water. When

the co-reactant is applied in a separate step either before or after the treatment with the aziridinyl compound, the solvent as that used in connection with the aziridine com-material may be miscible or immiscible with the solvent system from which the aziridinyl compound is applied. It has been observed that the pH of the treating solution may be varied within a considerable range. Generally, very high and very low pH ranges should be avoided since degradation of the wool can occur under extreme conditions. A pH range in general of 3.0 to about 9.0 is suitable with the range of 4.0 to 8.0 being preferred for most applications.

Methods of application of the polyfunctional compounds to the woolen textile not being critical, the treating solution can be applied by any suitable means including padding, spraying, dipping or the like. Excess solution is generally removed by wringing, squeezing, centrifuging or spinning. Thereafter, the woolen textile material is dried at a temperature ranging from ambient temperature to about 100° C., the range of 50° C. to 70° C. being particularly convenient. It is to be noted that the drying step is not essential to the overall efficiency of the process. After drying, the treated textile is cured by allowing it to stand at ambient temperature for several hours or preferably by heating for a few minutes at 110° C. to about 170° C. to complete the insolubilization reaction. The time required for the curing step varies with the particular reagent and the concentrations employed. It will be noted that the curing duration will be dependent upon the temperature, the higher temperatures requiring less curing time. Curing cycles of 3 to 15 minutes at 120° C. to 150° C. have been found to give excellent results in the majority of situations. The above ranges are indicative of suitable reaction conditions and are by no means considered limiting of the present invention.

Although the textile may be used without further treatment, it is generally preferred to wash the textile after the curing step with suitable detergent solutions, solvent scours or by any other desirable means in order to remove residual soluble unreacted chemicals. The textile material can thereafter be dyed by conventional procedures or subjected to other conventional chemical or mechanical finishing operations such as shearing, topping with softeners and other textile treatments designed to impart specific properties or behavior characteristics.

The following examples are illustrative of the process of the invention. Parts are by weight unless otherwise specified. The methods used in obtaining the test data given in the examples are as follows:

*Shrinkage.*—Measurement after laundering according to the following procedure: Samples ca. 18 x 18 inches with 10 x 10-inch markings laundered in an automatic home-type agitator washing machine at 41° C., using a 5-lb. load, detergent (Fab or Tide) and 15 minutes suds time. Washed samples were rinsed, extracted in the washer for the full cycle, dried flat on a horizontal screen and flat-bed pressed for 5 seconds at 135°-150° C. and conditioned for a minimum of 12 hours at 63 to 67% R.H. and 20-22° C. The samples were then measured for shrinkage in the warp and filling directions. Results reported in percent. The number of laundering-drying cycles is indicated by 5L or 10L, respectively.

*Flex abrasion resistance.*—ASTM-D-1175-61T. (Stoll Flex Abrader, ½ lb. head, 2 lbs. toggle). Results reported in cycles to break.

*Stiffness.*—Cantilever procedure. ASTM-D-1388-55T. Results reported in milligram-centimeters.

*Reflectance.*—ASTM-E97-55. Photovolt 610 and Search 6104, using the green tristimulus filter.

*Oil repellency.*—Minnesota Mining and Manufacturing Bulletin on Fluorochemical, Appendix A, pages 1-2. Measured after laundering (same washing procedure as for Shrinkage) and after dry cleaning (Minnesota Mining and Manufacturing Test Method for laboratory dry cleaning procedure, l.c. page 4).

*Tensile strength.*—ASTM—D—1682—59T, one-inch ravelled strip method. Reported in pounds.

*Fuzziness rating.*—The hairy appearance was expressed by the following numerical scale after brushing the fabric for 10 minutes on a testing machine:

- (1) Severe fuzzing
  - (2) Considerable fuzzing
  - (3) Moderate fuzzing
  - (4) Slight fuzzing
  - (5) No (or negligible) fuzzing

Fuzzing caused by laundering was rated after machine washing at 105° F. and tumble drying (12 such cycles in Example XXII, 10 in Example XXIII).

**Flat frosting rating.**—Variation in appearance of colored fabric caused by concentrated localized *abrasive wear*. (Flexing is not used in flat frosting.) The AATCC Gray Scale for Evaluating Changes in Color was used in applying the following rating scale to the descriptive meanings:

- (1) Severe change
  - (2) Considerable change
  - (3) Moderate change
  - (4) Slight change
  - (5) No (or negligible) change

polymer has three of the following groups per molecule attached to a polypropylene ether glycol backbone:



The full structure is believed to be:



wherein  $x+y+z=50$ .

The solution contained 4% ITP-63A and was applied to the sample by using a laboratory padder and setting the rolls of the padder at such a pressure as to obtain a wet pickup of about 110%.

20 The fabric sample so treated was framed at the original dimensions and dried at 65° C., then cured for 5 minutes at 135° C. in a forced-draft oven. The cured fabric was rinsed in toluene, dioxane, and finally in water. The sample was then again framed to the original dimensions and 25 held. The test results obtained were as follows:

25 dried. The test results obtained were as follows:

| Percent Reagent applied OWF <sup>1</sup> | Percent W.G. | Percent shrinkage after - |      |      |      | Flex<br>abr. res.,<br>cycles -W. | Reflec-<br>tance |
|------------------------------------------|--------------|---------------------------|------|------|------|----------------------------------|------------------|
|                                          |              | 5L                        |      | 10L  |      |                                  |                  |
|                                          |              | W                         | F    | W    | F    |                                  |                  |
| 4.4                                      | 3.9          | 1.5                       | 2.0  | 1.5  | 2.5  | 550                              | 59               |
| Untreated control                        |              | 18.0                      | 14.5 | 20.5 | 17.5 | 625                              | 60               |

### LOWE=On Weight of Fabric.

NOTE.—W.G.=Percent Weight Gain due to Treatment.

### EXAMPLE II

Dimensional stabilization of wool fabric by treatment with the imine-terminated polymer of Example I and a polyamine

45 Samples of plain weave 100% woolen fabric in the ready-to-dye state were treated with mixtures of ITP-63A and polyamines by padding from a 4:1 benzene-DMF solution. The equivalent ratio of the imine-terminated polymer to the amine co-reactant was 1:1, with the weight ratio as specified below. The steps of the treatment were 50 as described in Example I, except that the wet pickup was about 120%.

| Amine   | In the pad solution         |                    | Percent               |                 |
|---------|-----------------------------|--------------------|-----------------------|-----------------|
|         | Percent<br>amine            | Percent<br>ITP-63A | Total<br>reag.<br>OWF | Percent<br>W.G. |
| Sample: |                             |                    |                       |                 |
| B.....  | Tetraethylene<br>pentamine. | 0.11               | 3.49                  | 4.42            |
| C.....  | Diethylenetri-<br>amine.    | 0.10               | 3.50                  | 4.24            |
| D.....  | 1,3-diaminopro-<br>pane.    | 0.11               | 3.49                  | 4.28            |
| E.....  | 1,6-diaminohexane.          | 0.16               | 3.44                  | 4.31            |

The properties of the treated samples were as follows:

| Sample:           | Percent<br>shrinkage<br>10L |      | Stiff-<br>ness W,<br>mg.-cm. | Flex abr.,<br>cycles-W | Reflec-<br>tance |
|-------------------|-----------------------------|------|------------------------------|------------------------|------------------|
|                   | W                           | F    |                              |                        |                  |
| B                 | 1.5                         | 2.5  | 223                          | 825                    | 57               |
| C                 | 1.0                         | 2.5  | 171                          | 700                    | 57               |
| D                 | 1.0                         | 2.0  | 172                          | 625                    | 59               |
| E                 | 1.0                         | 2.5  | 195                          | 775                    | 60               |
| Untreated control | 18.0                        | 14.5 | 92                           | 625                    | 60               |

**13**  
**EXAMPLE III**

Dimensional stabilization of woolen fabric with a propylene imine-terminated polymer employed in Example I and a polycarboxylic acid

**14**

(4% toluene, 0.4% Triton X-100 nonionic surface active agent, 95.6% water) at room temperature for 5 minutes, then washed in water at 100° F. for 15 minutes, rinsed in cold water and dried on frames.

5 The properties of the treated samples were as follows:

| Fabric                         | Percent polymer<br>OWF | Percent<br>W.G. | Percent shrinkage |       |       |       |                       |                            |
|--------------------------------|------------------------|-----------------|-------------------|-------|-------|-------|-----------------------|----------------------------|
|                                |                        |                 | 5L                |       | 10L   |       | Stiffness,<br>mg.-cm. | Flex. abr.<br>res., cycles |
|                                |                        |                 | W                 | F     | W     | F     |                       |                            |
| Plain weave, woolen RTD*       | 3.7                    | 3.1             | 2.5               | 2.5   | 2.5   | 3.0   | 136                   | 600                        |
| Untreated RTD                  | 19.0                   | 17.5            | 28.5              | 26.0  | 1.5   | 2.0   | 103                   | 475                        |
| Twill weave, woolen RTD        | 3.6                    | 2.7             | 1.5               | 2.0   | 1.5   | 2.0   | 203                   | 775                        |
| Untreated                      | 20.0                   | 18.5            | 27.5              | 26.0  | 6.5   | 6.5   | 164                   | 575                        |
| Twill weave, woolen dyed green | 3.6                    | 2.9             | 5.0               | 5.5   | 6.5   | 6.5   | 171                   | 400                        |
| Untreated dyed                 | 23.5                   | 20.0            | 30.0              | 25.5  | ----- | ----- | 105                   | 525                        |
| Twill weave, worsted           | 3.2                    | 2.5             | 3.5               | 3.5   | ----- | ----- | 176                   | 3,400                      |
| Untreated RTD                  | 33.5                   | 30.0            | -----             | ----- | ----- | ----- | 165                   | 4,190                      |

\*RTD=Ready-to-Dye.

Example II was repeated, but polycarboxylic acids were used as co-reactants in the treating solution in place of the amino co-reactants.

| Sample: | Polycarboxylic acid | In the pad solution |                 |         | Percent total<br>reag.<br>OWF | Percent<br>W.G. |
|---------|---------------------|---------------------|-----------------|---------|-------------------------------|-----------------|
|         |                     | Percent poly-       | Percent         | Percent |                               |                 |
|         |                     | carboxylic acid     | carboxylic acid | ITP-63A |                               |                 |
| F       | Citric              | 0.18                | 3.42            | 4.17    | 5.3                           |                 |
| G       | Adipic              | 0.20                | 3.40            | 4.14    | 5.3                           |                 |
| H       | Sebacio             | 0.27                | 3.33            | 4.31    | 5.5                           |                 |

The properties of the treated samples were as follows:

| Sample: | Percent shrinkage |     |     |     |                         |                                      |
|---------|-------------------|-----|-----|-----|-------------------------|--------------------------------------|
|         | 5L                |     | 10L |     | Stiffness W,<br>mg.-cm. | Resistance to flex abr.,<br>W cycles |
|         | W                 | F   | W   | F   |                         |                                      |
| F       | 1.0               | 3.0 | 1.0 | 3.0 | 167                     | 725                                  |
| G       | 1.0               | 2.0 | 1.0 | 2.0 | 143                     | 675                                  |
| H       | 1.5               | 2.0 | 1.5 | 2.0 | 167                     | 650                                  |

**EXAMPLE IV**

Dimensional stabilization of woolen fabrics of various weaves using the polymer employed in Example I

Samples of plain weave and twill weave woolen fabric

25 Samples of dyed plain weave 100% woolen and twill weave worsted fabric were treated with a mixture of ITP-63A aqueous emulsion (preparation of the emulsion is described in Example IV) and of a fluorochemical emulsion, Scotchgard FC-208 (product of Minnesota Mining & Manufacturing Co.), which is a nonionic latex of a modified fluorinated acrylic polymer of the type polyperfluoroalkyl acrylate using a laboratory padder and setting the rolls at such a pressure as to give 90-116% wet pickup. The fabric samples so treated were framed and 30 dried at 150° F., then cured at 320° F. for 5 minutes in a forced-draft oven. The cured fabric samples were washed and dried in the manner described in Example IV. The properties of the treated samples were as follows:

TREATMENT

| Fabric           | Percent polymer<br>OWF | Percent Scotch- | Percent<br>W.G. |
|------------------|------------------------|-----------------|-----------------|
| Sample: A Woolen | 4.0                    | 2.2             | 4.3             |
| B do             | 2.9                    | 2.3             | 3.0             |
| C Worsted        | 3.4                    | 1.8             | 3.9             |

TESTING

| Sample:               | Percent shrinkage |     |      |      |                         |                                | Oil Repellency |    |       |        |                    |  |
|-----------------------|-------------------|-----|------|------|-------------------------|--------------------------------|----------------|----|-------|--------|--------------------|--|
|                       | 1L                |     | 5L   |      | Stiffness W,<br>mg.-cm. | Flex abr.<br>res., W<br>cycles | Orig.          | 1L |       |        | 2 Dry<br>cleanings |  |
|                       | W                 | F   | W    | F    |                         |                                |                | 1L | 5L    | 1 D.C. | 2 D.C.             |  |
| (1) A                 | 1.0               | 2.5 | 2.0  | 3.5  | 144                     | 775                            | 100+           | 90 | 70/80 | 80/90  | 70                 |  |
| (2) B                 | 2.0               | 3.0 | 3.5  | 4.5  | 116                     | 525                            | 100+           | 90 | 70    | 80     | 50                 |  |
| (3) Untreated woolen  | 8.5               | 6.0 | 14.5 | 12.5 | 84                      | 450                            | 0              |    |       |        |                    |  |
| (4) C                 | 2.0               | 2.5 | 5.5  | 6.0  | 195                     | 3,700                          | 100            |    |       |        |                    |  |
| (5) Untreated worsted | 9.5               | 8.5 | 24.5 | 22.0 | 131                     | 3,300                          | 0              |    |       |        |                    |  |

and of twill weave worsted fabric were treated with an aqueous emulsion of ITP-63A.

The emulsion was prepared by mixing 120 parts of a 50% xylene solution of ITP-63A with 10 parts of the nonionic surface active agent, t-octylphenylmona(ethyleneoxy)ethanol (Triton X-100, a product of Rohm & Haas Co.), dissolved in 20 parts of water with stirring. The emulsion obtained in this manner was diluted with water to the desired concentration. The fabric samples were treated with the diluted emulsion using a laboratory padder, setting the rolls at such a pressure to give 80-100% wet pickup.

The fabric samples so treated were framed to the original dimension and dried at 150° F., then cured for 5 minutes at 300° F. in a forced-draft oven. The cured fabric samples were rinsed in an aqueous toluene emulsion

60 generally, the above mentioned fluorochemical finishes are believed to be made from monomers having the basic formula  $R_fCH_2O-COCH=CH_2$  where  $R_f$  can vary from  $-C_2F_5$  to  $-C_9F_{19}$ , for example.

EXAMPLE VI

65 Hydroextraction of dimensionally stabilized woolen fabric

Samples of plain weave 100% woolen fabric were immersed for 10 seconds into a 4% aqueous emulsion of ITP-63A (preparation of the emulsion is described in Example IV). The fabric samples so treated were hydroextracted for 10 seconds and then dried in a home-type tumble dryer at 200-210° F. for 40 to 80 minutes. The treated samples were then washed and dried in the manner described in Example IV.

The properties of the treated samples were as follows:

| Percent ITP in the bath | Percent ITP, OFW | Drying Time in minutes | Percent shrinkage |     |      |      |
|-------------------------|------------------|------------------------|-------------------|-----|------|------|
|                         |                  |                        | IL                |     | 5L   |      |
| W                       | F                | W                      | F                 | W   | F    |      |
| 4.0                     | 4.1              | 80                     | 1.0               | 0.5 | 1.5  | 0.5  |
| 2.0                     | 1.8              | 40                     | 1.5               | 0.5 | 5.5  | 2.5  |
| 2.0                     | 1.8              | 60                     | 0.5               | 0.5 | 0.5  | 0.5  |
| 2.0                     | 1.8              | 80                     | 0.5               | 0.5 | 0.5  | 0.5  |
| Unreated control        |                  |                        | 8.5               | 6.0 | 14.5 | 12.5 |

### EXAMPLE VII

Dyeing of woolen fabrics dimensionally stabilized with aqueous emulsion of polymers employed in Example IV

Samples of twill weave 100% woolen fabric in ready-to-dye state were treated with an aqueous ITP-63A emulsion (percent polymer OFW: 4%) according to the procedure described in Example IV. After the shrinkproofing treatment, the samples were dyed with 0.75% and 3.0% Du Pont Anthraquinone Blue SWF (C.I. No. 62055, C.I., Acid Blue 25) acid dye and also with 0.75% capracyl Red BB (Color Index name C.I. Acid Red 178) pre-metallized dyestuff. In each case, untreated wool samples were dyed in the same dye bath with the treated samples. Testing of the samples before and after dyeing gave the following results:

| Color          | Percent shrinkage |      |      |      |                 |                             |                   |                          |
|----------------|-------------------|------|------|------|-----------------|-----------------------------|-------------------|--------------------------|
|                | 5L                |      | 10L  |      | Tensile str., W | Res. to flex abr., W cycles | Stiffness, mg.-cm | Percent Total Reag. W.G. |
|                | W                 | F    | W    | F    |                 |                             |                   |                          |
| Sample:        |                   |      |      |      |                 |                             |                   |                          |
| A-1, treated   | RTD               | 3.0  | 3.5  |      | 20              | 900                         | 231               |                          |
| A-2, untreated | RTD               | 22.5 | 22.5 | 27.0 | 26.0            | 20                          | 775               | 142                      |
| B-1, treated   | Light Red         | 2.5  | 3.0  | 2.5  | 3.0             | 20                          | 450               | 249                      |
| B-2, untreated | do                | 15.5 | 18.5 | 18.5 | 22.5            | 17                          | 400               | 119                      |
| C-1, treated   | Dark Red          | 2.0  | 2.5  | 2.0  | 2.5             | 19                          | 415               | 231                      |
| C-2, untreated | do                | 18.0 | 19.0 | 22.5 | 23.5            | 17                          | 325               | 167                      |
| D-1, treated   | Light Blue        | 1.5  | 1.0  | 1.5  | 1.5             | 21                          | 675               | 218                      |
| D-2, untreated | do                | 15.5 | 17.5 | 20.0 | 23.5            | 20                          | 575               | 147                      |
| E-1, treated   | Dark Blue         | 2.0  | 0.5  | 2.0  | 1.0             | 22                          | 775               | 160                      |
| E-2, untreated | do                | 16.0 | 17.5 | 19.5 | 22.5            | 20                          | 800               | 231                      |

The depth of shade and the brightness of color obtained in dyeing the shrinkproofed and the untreated samples were fully comparable and the treated samples dyed as evenly as the untreated.

The colorfastness of the dyed samples shown in the preceding table were as follows: In each case the "1" samples were dyed after shrinkproofing and the "2" samples were dyed in the untreated state.

| Washfastness at 105° F.—alteration of shade | Colorfastness to— |          |     |              |          |   |
|---------------------------------------------|-------------------|----------|-----|--------------|----------|---|
|                                             | Light, 20 hrs.    | Crocking |     | Perspiration |          | W |
|                                             |                   | Dry      | Wet | Acid         | Alkaline |   |
| Sample:                                     |                   |          |     |              |          |   |
| B-1                                         | 3/4               | 2/3      | 3   | 5            | S        | S |
| B-2                                         | 4/5               | 5        | 5   | 4            | S        | S |
| C-1                                         | 3/4               | 2/3      | 2   | 4            | U        | U |
| C-2                                         | 4                 | 4        | 3   | 3            | U        | U |
| D-1                                         | 2                 | 2/3      | 4   | 5            | U        | U |
| D-2                                         | 2                 | 2        | 5   | 5            | U        | U |
| E-1                                         | 2                 | 2        | 2/3 | 4            | U        | U |
| E-2                                         | 2                 | 2        | 5   | 2/3          | U        | U |

NOTE.—S=Satisfactory; U=Unsatisfactory.

### EXAMPLE VIII

Dimensional stabilization of woolen fabric with another type of imine-terminated polymer and a polyamine

Samples of twill weave 100% woolen fabric in the ready-to-dye state were treated with mixtures of an imine-terminated polymer marketed by the Interchemical Corp. under the trade name of ITP-43 and having an average molecular weight of about 2600, and an aziridinyl content of about 0.65 meq./g., and with the polyamines shown in the table as co-reactants. The ITP-43 polymer

75

### 16

is a linear polyester (molecular weight of approximately 2100, made from a diol and a dibasic acid of the type shown in Formula IV) containing the following imine group attached to the backbone:



10 A 5:4:1 DMF-toluene-acetone solution was used to prepare the treating solution used for the application. The equivalent ratio of the imine terminated polymer to the polyamine was in each case 1:1 with the weight ratio indicated below.

15 The treatment was carried out in the manner described in Example I.

| Amine                           | Percent Amine pad solution | Percent Total ITP-43 | Percent Total Reag. OFW | Percent W.G. |
|---------------------------------|----------------------------|----------------------|-------------------------|--------------|
|                                 |                            |                      |                         |              |
| Sample:                         |                            |                      |                         |              |
| B..... Tetraethylene-pentamine. | 0.11                       | 3.7                  | 4.9                     | 6.3          |
| C..... Diethylenetriamine.      | 0.10                       | 3.7                  | 4.9                     | 3.3          |
| D..... 1,3-diaminopropane.      | 0.11                       | 3.7                  | 4.9                     | 1.8          |
| E..... 1,6-diamino-hexane.      | 0.16                       | 3.6                  | 4.9                     | 1.7          |

The physical properties of the treated samples were as follows:

45

| Sample:                | Percent Shrinkage-5L |      | Flex Abr. Res., W Cycles | Stiffness—W, mg.-cm. |
|------------------------|----------------------|------|--------------------------|----------------------|
|                        | W                    | F    |                          |                      |
| B.....                 | 2.0                  | 2.0  | 1,225                    | 460                  |
| C.....                 | 3.0                  | 2.5  | 1,100                    | 439                  |
| D.....                 | 9.5                  | 11.5 | -----                    | -----                |
| E.....                 | 11.5                 | 10.0 | -----                    | -----                |
| Untreated control..... | 19.5                 | 15.5 | 575                      | 164                  |

55

### EXAMPLE IX

Dimensional stabilization of woolen fabrics with the imine-terminated polymer of Example VIII and a polycarboxylic acid

60 Example VIII was repeated but, in place of the polyamines, polycarboxylic acids were used as co-reactants with ITP-43.

65

| Polycarboxylic acid | Percent Polycarboxylic acid in the pad bath | Percent Total ITP-43 | Percent Total reag. OFW | Percent W.G. |
|---------------------|---------------------------------------------|----------------------|-------------------------|--------------|
|                     |                                             |                      |                         |              |
| Sample:             |                                             |                      |                         |              |
| A..... None.....    |                                             | 3.8                  | 4.8                     | 1.9          |
| F..... Citric.....  | 0.18                                        | 3.62                 | 5.0                     | 1.9          |
| G..... Adipic.....  | 0.20                                        | 3.60                 | 4.9                     | 1.8          |
| H..... Sebacic..... | 0.27                                        | 3.53                 | 4.9                     | 1.9          |

## EXAMPLE X

## Dimensional stabilization of a dyed wool fabric

A 100-yd. length of 100% woolen fabric of 60-inch width, twill weave, dyed bright red, was treated by padding with an aqueous emulsion containing 8% of the ITP-63A imine-terminated polymer. The wet pickup was 60%. The fabric was dried on a frame, cured for 6 minutes at 275° F., thoroughly washed at 110° F. in a non-ionic detergent solution, dried and sheared to enhance its appearance. The properties of the red fabric before and after the shrinkproofing treatment described are tabulated below:

|                                         | Before treatment | After treatment |
|-----------------------------------------|------------------|-----------------|
| Count (W x F)                           | 36 x 32          | 37 x 33         |
| Percent shrinkage in relaxation (W x F) | 5.0 x 4.3        | 2.0 x 2.5       |
| Total after 1L                          | 11.5 x 7.5       | 2.0 x 2.5       |
| Total after 5L                          | 22.0 x 17.0      | 2.5 x 2.8       |
| Total after 10L                         | 25.0 x 19.5      | 3.0 x 3.0       |
| Tensile strength, W lbs                 | 19               | 21              |
| Tear strength, W lbs                    | 2.8              | 2.7             |
| Flex abr. res., cycles                  | 490              | 550             |
| Stiffness, mg.-cm.                      | 132              | 134             |
| Weight (oz./sq. yd.)                    | 7.29             | 7.48            |
| Colorfastness:                          |                  |                 |
| To light:                               |                  |                 |
| 20 hrs                                  | 5                | 5               |
| 40 hrs                                  | 4/5              | 4/5             |
| To wash                                 | 4/5              | 4/5             |
| To crocking:                            |                  |                 |
| Dry                                     | 5                | 5               |
| Wet                                     | 3                | 5               |
| To perspiration:                        |                  |                 |
| Acid                                    | 3                | 4               |
| Alkali                                  | 3                | 4               |

## EXAMPLE XI

Preparation of a polyfunctional compound having (1) a polyester chain as its backbone and (2) terminal 1-aziridinyl radicals

solved in 100 grams of methylene chloride. Ethylenimine (10.7 grams, 0.25 equivalent), dissolved in 100 ml. of methylene chloride, was added dropwise to the stirred solution in the flask at 25 to 28° C. The addition was completed in 1 hour, and the reaction solution remained homogeneous. Stirring was continued for 5 hours longer. Then solvent and unreacted ethylenimine were distilled off in vacuo, leaving behind the addition product, ethylenimine-terminated polyester, as a waxy solid.

The product was analyzed for aziridinyl content by a procedure modified after that of Allan and Seaman, Anal. Chem., vol. 27, page 540 (1955). It was found to have an aziridinyl content of 1.73 milliequivalents per gram, as compared with 2.06 millieq./g. theoretically possible. The conversion, based on aziridinyl activity, was 84%. The product was very soluble in toluene and in N,N-dimethylformamide.

## EXAMPLE XII

Preparation of a polyfunctional compound having (1) a polyester chain as its backbone and (2) terminal 2-methyl-1-aziridinyl radicals

Isocyanate-terminated polyester as in Example XI



Propylenimine-terminated polyester

A 1-liter 3-neck flask equipped with a stirrer, a thermometer, a reflux condenser, and a dropping funnel was charged with 14.2 grams (0.26 equivalent) of propylenimine dissolved in 50 ml. of methylene chloride. Isocyanate-terminated polyester (100 grams, 0.23 equivalent) dissolved in 150 ml. of methylene chloride was added dropwise to the stirred solution at 25 to 28° C. (The isocyanate-terminated polyester was of the same composition as that used as starting material in Example XI, but 40 both the order of addition and the alkylenimine were



Isocyanate-terminated polyester, wherein  $v=3-4$  and  $n$  is about 6.

different from those of Example XI.) The addition was completed in 1 hour, and the reaction solution remained



1-aziridinyl-terminated polyester.

The isocyanate-terminated polyester used as the starting material had an isocyanate content of 9.5% and was obtained under the registered trademark of Isofoam L-128 from Isocyanate Products, Inc., Wilmington, Del.

A 1-liter 3-neck flask equipped with a stirrer, a thermometer, a reflux condenser, and a dropping funnel was charged with 100 grams (0.23 equivalent based on isocyanate content) of isocyanate-terminated polyester dis-

70 homogeneous. Stirring was continued for 5 hours longer. Then solvent and unreacted propylenimine were distilled off in vacuo, leaving behind the addition product, propylenimine-terminated polyester, as a waxy solid.

Using the analytical method cited in Example XI, the product was found to have 1.60 milliequivalents of aziridinyl nitrogen per gram. Based on that, the extent of conversion was 80%. This product was very soluble in toluene and in N,N-dimethylformamide.

**13**  
**EXAMPLE XIII**

Preparation of a polyfunctional compound having (1) a polybutadiene chain as its backbone and (2) terminal 1-aziridinyl radicals

### *First stage:*



### Isocyanate-terminated polybutadiene (VI)

### *Second stage:*



### 1-Aziridinyl-terminated polybutadiene

The hydroxyl-terminated polybutadiene used as the starting material had a hydroxyl content of 0.80 milliequivalent per gram, an iodine number of 395, and an average molecular weight of  $3250 \pm 250$ . The polymer was supplied under the trade name Poly B-D Liquid Resin R-15M by Sinclair Petrochemicals, Inc. Prior to use, the resin was kept in vacuo in a slowly rotating flask for several hours to strip off moisture.

The first stage of the process consisted of converting the hydroxyl-terminated polybutadiene into isocyanate-terminated polybutadiene. A 2-liter 3-neck flask equipped with a stirrer, a thermometer, a gas inlet tube, and a dropping funnel was charged with 200 grams of the hydroxyl-terminated polybutadiene dissolved in 200 grams of methylene chloride. Toluene diisocyanate (43.6 grams, 0.25 mole of "2,4" and "2,6" isomers in the ratio of 80/20) was added while a stream of nitrogen was passed into the solution and the temperature was maintained at 20° C. After the addition, the solution was stirred at 25–28° C. for 8 hours.

Next, the *second stage* of adding terminal 1-aziridinyl radicals was carried out. Ethylenimine (12.9 grams, 0.30 mole), dissolved in 100 grams of methylene chloride, was added dropwise to the stirred solution. The addition was completed in 2.5 hours, during which time the temperature of the reaction was maintained at 25° C. The solution was stirred for 4 hours longer. Then solvent and unreacted ethylenimine were distilled off in *vacuo*. The product (223 grams) which remained was a light-brown viscous liquid.

Using the analytical method cited in Example XI, the product was found to have 1.00 milliequivalent of aziridinyl per gram, as compared with 0.97 millieq./g. expected. The product, ethylenimine-terminated polybutadiene, was very soluble in toluene, benzene, tetrahydrofuran and carbon tetrachloride.

#### EXAMPLE XIV

Preparation of a polyfunctional compound having (1) A polybutadiene chain as its backbone and (2) Terminal 2-methyl-1-aziridinyl radicals



### Propylenimine-terminated polybutadiene

First.—A 500-ml. flask equipped as in Example XIII was charged with 85.3 grams of the hydroxyl-terminated polybutadiene dissolved in 50 grams of methylene chloride. Toluene diisocyanate (18.5 grams, 0.16 mole of

5

*Second.*—Propylenimine (6.70 grams, 0.18 mole), dissolved in 50 grams of methylene chloride, was added dropwise to the stirred solution during a 3-hour period. The solution was stirred for 4 hours longer. Then solvent and unreacted propylenimine were distilled off in vacuo. The product which remained was a light-brown liquid.

Using the analytical method cited in Example XI, the product was found to have 0.90 milliequivalent of azidinyl nitrogen per gram, as compared with 0.97 millieq./g. theoretically possible. The product, propyl-elimine-terminated polybutadiene was very soluble in toluene.

### EXAMPLE XV

## Enhancement of surface characteristics of 70:30 rayon-wool fabric by imine-terminated polymer

Plain-weave fabric woven from a 70:30 blend of high-modulus high-tenacity rayon and wool was treated with the propylenimine-terminated polymer identified in Example I so that the reagent applied was 4%, based on the weight of the fabric. The fabric specimen so treated was framed at the original dimensions and dried at 150° F. (in approximately 10 minutes), then cured for 6 minutes at 275° F. The cured fabric was scoured to remove unreacted reagent by using an emulsion formulated from 4 parts of toluene, 0.4 part of Triton X-100 (emulsifying agent identified in Example IV), and 95.6 parts of water. Then the fabric specimen was again framed to the original dimensions and dried. The following results, along with those on an untreated fabric sample used as the control, clearly show that the treatment enhanced surface characteristics, and even improved the strength somewhat.

|                   | Fuzziness rating | Tensile strength, lb. (1-inch strip, F) | Flex abrasion res., cycles (1-lb. head-weight, 4-lb. toggle tension, W) |
|-------------------|------------------|-----------------------------------------|-------------------------------------------------------------------------|
| Treated specimen  | 4                | 61                                      | 1 555                                                                   |
| Untreated control | 2                | 56                                      | 2 260                                                                   |

75 <sup>1</sup>To web. <sup>2</sup>To break.

**21**  
**EXAMPLE XVI**

Control imparted on shrinkage and fuzziness to 50:50  
wool-rayon fabric by imine-terminated polymer

Plain-weave fabric woven from a 50:50 blend of wool  
and rayon was treated with the propylenimine-terminated  
polymer identified in Example I so that the reagent ap-

**22**

framed at the original dimensions and dried at 150° F.  
All samples were cured for 5 minutes. The cured fabric  
was rinsed in toluene, then in p-dioxane and finally in  
water containing 0.4% Triton X-100 (identified in Ex-  
ample IV). The samples were again framed to the origi-  
nal dimensions and dried. Excellent dimensional stabiliza-  
tion was achieved, as borne out by the following results:

|                   | Percentages on<br>wt. of bath |      | Wet<br>pickup,<br>percent | Total<br>add-on,<br>percent on<br>weight of<br>fabric | Curing<br>temp.,<br>° F.<br>(time =<br>5 mins.) | Shrinkage, percent |      | Flex abras.<br>( $\frac{1}{2}$ lb. x<br>2 lb.),<br>No L,<br>(warp) |      | Stiffness,<br>mg.-cm.,<br>No L,<br>(warp) |
|-------------------|-------------------------------|------|---------------------------|-------------------------------------------------------|-------------------------------------------------|--------------------|------|--------------------------------------------------------------------|------|-------------------------------------------|
|                   | Reagent                       | TEPA |                           |                                                       |                                                 | 5L                 | 10L  | W                                                                  | F    |                                           |
| <b>Sample:</b>    |                               |      |                           |                                                       |                                                 |                    |      |                                                                    |      |                                           |
| Y-1               | 5.0                           | None | 109                       | 5.4                                                   | 275                                             | 0.5                | 1.0  | 0.5                                                                | 1.0  | -----                                     |
| Y-2               | 5.0                           | None | 107                       | 5.3                                                   | 325                                             | 1.0                | 1.5  | 1.5                                                                | 1.5  | -----                                     |
| Z-1               | 5.0                           | 0.5  | 107                       | 5.3                                                   | 275                                             | 1.5                | 1.0  | 2.0                                                                | 1.5  | -----                                     |
| Z-2               | 5.0                           | 0.5  | 108                       | 5.4                                                   | 325                                             | 1.5                | 2.0  | 1.5                                                                | 2.0  | -----                                     |
| A                 | 5.0                           | None | 127                       | 6.3                                                   | 275                                             | 1.5                | 1.5  | 2.0                                                                | 2.5  | 970                                       |
| B                 | 4.0                           | None | 128                       | 5.1                                                   | 275                                             | 2.5                | 2.0  | 2.5                                                                | 3.0  | 880                                       |
| C                 | 3.0                           | None | 127                       | 3.8                                                   | 275                                             | 1.5                | 3.5  | 2.5                                                                | 4.0  | 900                                       |
| D                 | 2.0                           | None | 129                       | 2.6                                                   | 275                                             | 3.5                | 2.5  | 4.5                                                                | 3.5  | 875                                       |
| E                 | 5.0                           | 0.5  | 124                       | 6.8                                                   | 275                                             | 1.0                | 2.5  | 1.5                                                                | 3.0  | 975                                       |
| F                 | 4.0                           | 0.4  | 124                       | 5.5                                                   | 275                                             | 2.5                | 1.5  | 2.5                                                                | 2.5  | 1,050                                     |
| G                 | 3.0                           | 0.3  | 124                       | 4.1                                                   | 275                                             | 2.5                | 2.5  | 3.5                                                                | 3.0  | 970                                       |
| H                 | 2.0                           | 0.2  | 138                       | 2.8                                                   | 275                                             | 4.5                | 3.0  | 5.0                                                                | 4.0  | 900                                       |
| Untreated control |                               |      |                           |                                                       |                                                 | 27.0               | 21.5 | 32.5                                                               | 27.5 | 850                                       |
|                   |                               |      |                           |                                                       |                                                 |                    |      |                                                                    |      | 130                                       |

plied was 3.5% based on the weight of the fabric. Con-  
ditions of framing, drying, curing, scouring, reframing,  
and redrying were those of Example XV. The following  
results, and those of the untreated fabric sample used  
as the control, show much more satisfactory control of  
shrinkage and of fuzziness for the treated specimen.

|                   | Shrinkage, percent (Tumble dried<br>at 105° F.) |      |      |      |       |       | Fuzziness<br>rating |  |
|-------------------|-------------------------------------------------|------|------|------|-------|-------|---------------------|--|
|                   | 1L                                              |      | 5L   |      | 10L   |       |                     |  |
|                   | W                                               | F    | W    | F    | W     | F     |                     |  |
| Treated specimen  | 4.0                                             | 5.0  | 4.0  | 5.0  | 4.5   | 5.5   | 4                   |  |
| Untreated control | 14.0                                            | 17.0 | 16.5 | 19.5 | ----- | ----- | 2                   |  |

|                   | Percentages on<br>weight of bath |      | Wet<br>pickup,<br>percent | Total<br>add-on,<br>percent on<br>weight of<br>fabric | Curing<br>temp.,<br>° F.<br>(time =<br>5 mins.) | Shrinkage, percent |      | Flex abras.<br>( $\frac{1}{2}$ lb. x<br>2 lb.),<br>No L,<br>(warp) |      | Stiffness,<br>mg.-cm.,<br>No L,<br>(warp) |
|-------------------|----------------------------------|------|---------------------------|-------------------------------------------------------|-------------------------------------------------|--------------------|------|--------------------------------------------------------------------|------|-------------------------------------------|
|                   | Reagent                          | TEPA |                           |                                                       |                                                 | 5L                 | 10L  | W                                                                  | F    |                                           |
| <b>Sample:</b>    |                                  |      |                           |                                                       |                                                 |                    |      |                                                                    |      |                                           |
| A-1               | 5.0                              | None | 127                       | 6.3                                                   | 275                                             | 1.0                | 2.0  | 1.5                                                                | 2.5  | -----                                     |
| A-2               | 5.0                              | None | 126                       | 6.3                                                   | 325                                             | 1.0                | 1.5  | 1.5                                                                | 1.5  | -----                                     |
| B-1               | 5.0                              | 0.5  | 123                       | 6.1                                                   | 275                                             | 1.5                | 1.5  | 1.5                                                                | 2.0  | -----                                     |
| B-2               | 5.0                              | 0.5  | 120                       | 6.0                                                   | 325                                             | 0.5                | 3.0  | 1.0                                                                | 3.5  | -----                                     |
| C-1               | 3.0                              | None | 122                       | 3.7                                                   | 275                                             | 1.5                | 2.5  | 2.0                                                                | 3.0  | -----                                     |
| C-2               | 3.0                              | None | 118                       | 3.5                                                   | 325                                             | 1.5                | 1.5  | 2.0                                                                | 2.0  | -----                                     |
| D-1               | 2.9                              | 1.0  | 123                       | 3.6                                                   | 275                                             | 1.0                | 2.0  | 1.0                                                                | 2.0  | -----                                     |
| D-2               | 2.9                              | 1.0  | 120                       | 3.5                                                   | 325                                             | 1.5                | 1.0  | 1.5                                                                | 1.0  | -----                                     |
| Untreated control |                                  |      |                           |                                                       |                                                 | 25.0               | 22.5 | 32.0                                                               | 29.0 |                                           |

**EXAMPLE XVII**

Dimensional stabilization of woolen fabric by treatment  
with ethylenimine-terminated polybutadiene

Samples of plain-weave woolen fabric in the ready-  
to-dye state were treated with solutions of various con-  
centrations of the reagent prepared in Example XIII,

50 (B) *Pad - bath solvent: Toluene - dimethylformamide  
(5:1)*.—The procedure described under part A was fol-  
lowed, except that a 5:1 weight ratio of toluene-dimethyl-  
formamide was used instead of the 1:1 ratio, and lower  
concentrations of the reagent were used to establish its  
shrinkproofing efficiency. As before, shrinkage control was  
impressive, as shown by the following results.

|                   | Percentages on<br>wt. of bath |      | Wet<br>pickup,<br>percent | Total<br>add-on,<br>percent on<br>weight of<br>fabric | Curing<br>temp.,<br>° F.<br>(time =<br>5 mins.) | Shrinkage, percent |      | Flex abras.<br>( $\frac{1}{2}$ lb. x<br>2 lb.),<br>No L,<br>(warp) |      | Stiffness,<br>mg.-cm.,<br>No L,<br>(warp) |
|-------------------|-------------------------------|------|---------------------------|-------------------------------------------------------|-------------------------------------------------|--------------------|------|--------------------------------------------------------------------|------|-------------------------------------------|
|                   | Reagent                       | TEPA |                           |                                                       |                                                 | 5L                 | 10L  | W                                                                  | F    |                                           |
| <b>Sample:</b>    |                               |      |                           |                                                       |                                                 |                    |      |                                                                    |      |                                           |
| P                 | 3.0                           | None | 127                       | 3.8                                                   | 275                                             | 2.5                | 1.5  | 2.5                                                                | 1.5  | 900                                       |
| Q                 | 2.0                           | None | 123                       | 2.5                                                   | 275                                             | 2.0                | 2.5  | 2.0                                                                | 3.5  | 850                                       |
| R                 | 1.0                           | None | 121                       | 1.2                                                   | 275                                             | 2.5                | 2.5  | 2.5                                                                | 3.0  | 715                                       |
| S                 | 3.0                           | 0.6  | 128                       | 3.8                                                   | 275                                             | 1.0                | 2.0  | 1.0                                                                | 2.5  | 875                                       |
| T                 | 2.0                           | 0.4  | 123                       | 2.5                                                   | 275                                             | 3.0                | 2.5  | 3.0                                                                | 2.5  | 900                                       |
| U                 | 1.0                           | 0.2  | 121                       | 1.2                                                   | 275                                             | 6.5                | 6.0  | 8.5                                                                | 7.5  | 950                                       |
| Untreated control |                               |      |                           |                                                       |                                                 | 24.0               | 20.0 | 30.0                                                               | 27.5 | 675                                       |
|                   |                               |      |                           |                                                       |                                                 |                    |      |                                                                    |      | 90                                        |

namely, ethylenimine - terminated polybutadiene. Con-  
centrations and other details were shown in the accom-  
panying table. In preparing certain of the samples, tetra-  
ethylenepentamine (TEPA) was also used in the pad  
bath. The solvent was toluene-dimethylformamide (1:1).  
Solutions were applied to the fabric samples by means  
of a laboratory padder. After padding, the fabric was

70 Dimensional stabilization of woolen fabric by treatment  
with ethylenimine-terminated polyester

Samples of plain-weave woolen fabric in the ready-to-  
dye state were treated with solutions of various concen-  
trations of the reagent prepared in Example XI, namely,

ethylenimine-terminated polyester. In the treatment of some of the samples, a co-reactant was used, viz., tetra-ethylenepentamine (TEPA). The procedure followed that of Example XVII. Excellent shrinkage control resulted, as the following data show.

| Reagent           | TEPA | Percentages on weight of bath | Wet pickup, percent | Total add-on, percent on weight of fabric | Curing temp., °F. (time = 5 mins.) | Shrinkage, percent |      |      |      |
|-------------------|------|-------------------------------|---------------------|-------------------------------------------|------------------------------------|--------------------|------|------|------|
|                   |      |                               |                     |                                           |                                    | 5L                 |      | 10L  |      |
| W                 | F    | W                             | F                   |                                           |                                    |                    |      |      |      |
| <b>Sample:</b>    |      |                               |                     |                                           |                                    |                    |      |      |      |
| A-1               | 5.0  | None                          | 133                 | 6.6                                       | 275                                | 1.0                | 1.5  | 1.5  | 2.5  |
| A-2               | 5.0  | None                          | 133                 | 6.6                                       | 325                                | 0.5                | 2.0  | 1.0  | 2.0  |
| B-1               | 5.0  | 0.5                           | 133                 | 6.6                                       | 275                                | 1.5                | 3.0  | 2.0  | 3.0  |
| B-2               | 5.0  | 0.5                           | 131                 | 6.5                                       | 325                                | 1.0                | 2.0  | 1.5  | 3.0  |
| C-1               | 3.0  | None                          | 132                 | 4.0                                       | 275                                | 1.5                | 3.0  | 2.0  | 3.5  |
| C-2               | 3.0  | None                          | 130                 | 4.0                                       | 325                                | 1.0                | 3.0  | 1.5  | 3.5  |
| D-1               | 3.0  | 0.5                           | 134                 | 4.0                                       | 275                                | 1.0                | 3.0  | 2.5  | 4.0  |
| D-2               | 3.0  | 0.5                           | 13.0                | 3.9                                       | 325                                | 1.5                | 2.5  | 2.0  | 4.0  |
| Untreated control |      |                               |                     |                                           |                                    | 23.5               | 22.5 | 30.0 | 29.0 |

## EXAMPLE XX

Dimensional stabilization of woolen fabric by treatment with propylenimine-terminated polyester

Samples of plain-weave woolen fabric in the ready-to-dye state were treated with solutions of various concentrations of the reagent prepared in Example XII, namely, propylenimine-terminated polyester. In the treatment of some of the samples, a co-reactant was used, viz., tetra-ethylenepentamine (TEPA). The procedure followed that of Example XVII. The following results show that superior shrinkage control was obtained:

| Reagent           | TEPA | Percentages on wt. of bath | Wet pickup, percent | Total add-on, percent on weight of fabric | Curing temp., °F. (time = 5 mins.) | Shrinkage, percent |      |      |     | Flex abras. (1/2 lb. x 2 lb.), No L, (warp) | Stiffness, mg.-cm., No L, (warp) |
|-------------------|------|----------------------------|---------------------|-------------------------------------------|------------------------------------|--------------------|------|------|-----|---------------------------------------------|----------------------------------|
|                   |      |                            |                     |                                           |                                    | 5L                 |      | 10L  |     |                                             |                                  |
| W                 | F    | W                          | F                   |                                           |                                    |                    |      |      |     |                                             |                                  |
| <b>Sample:</b>    |      |                            |                     |                                           |                                    |                    |      |      |     |                                             |                                  |
| A                 | 3.0  | -----                      | 114                 | 3.4                                       | 275                                | 1.5                | 1.0  | 3.0  | 1.5 | 850                                         | 505                              |
| B                 | 2.0  | -----                      | 115                 | 2.3                                       | 275                                | 3.5                | 0.5  | 5.5  | 2.5 | 900                                         | 370                              |
| C                 | 1.0  | -----                      | 125                 | 1.2                                       | 275                                | 7.0                | 3.5  | 12.5 | 7.5 | 725                                         | 160                              |
| D                 | 3.0  | 0.6                        | 111                 | 3.3                                       | 275                                | 2.0                | 0.5  | 3.0  | 0.5 | 1,050                                       | 625                              |
| E                 | 2.0  | 0.4                        | 110                 | 2.2                                       | 275                                | 1.5                | None | 3.0  | 1.5 | 900                                         | 355                              |
| F                 | 1.0  | 0.2                        | 111                 | 1.1                                       | 275                                | 4.5                | 0.5  | 6.5  | 3.5 | 825                                         | 210                              |
| Untreated control |      |                            |                     |                                           |                                    | 27                 | 25   | 32   | 31  | 850                                         | 100                              |

## EXAMPLE XXI

Dimensional stabilization of woolen garments in the ready-to-wear condition by shrinkproofing agents applied as perchloroethylene solutions

Identical knitted wool sweaters were impregnated with perchloroethylene solutions of the imine-terminated polymer identified in Example I and designated as ITP 63-A below. Excess impregnating solution was centrifuged out of the sweaters in a hydroextractor. Processing details are tabulated below, followed by data on shrinkage occurring during processing and repeated laundering:

Improvement of dyed acrylic-wool blends by imine-terminated polymer, particularly with respect to control of fuzziness and resistance to abrasion  
5 Each of three 30-yard lengths of colored fabrics repre-

senting various acrylic-wool blends identified in the accompanying table was padded with a dispersion formulated as follows: First, ITP-63A (the imine-terminated polymer described in Example I) was dissolved in an equal weight of xylene, and a thick emulsion was prepared by mixing 80 parts of that solution with 20 parts of a 2:1 blend of water and Triton X-100 (identified in Example IV). Hence, the concentration of ITP-63A in the thick emulsion was 40%. Next, an approximately 3.9% dispersion of ITP-63A was made by blending 90 pounds of said thick emulsion and 100 gallons (approximately 830 pounds) of water.

| Sweater specimen | Percent of shrink-proofer in perchloroethylene | Time of hydro-extraction, seconds | Wet pickup, percent | Solids, percent on weight of fabric | Tumble drying (curing) time, minutes | Other conditions applied prior to measuring process shrinkage     |                |                                       |  |
|------------------|------------------------------------------------|-----------------------------------|---------------------|-------------------------------------|--------------------------------------|-------------------------------------------------------------------|----------------|---------------------------------------|--|
|                  |                                                |                                   |                     |                                     |                                      | 15-min. wash in toluene water 4:96 at 105° F., then tumble-dried. | Same as for W. | 1 wash at 140° F.; then tumble-dried. |  |
| W                | 10% of ITP-63A                                 | 7                                 | 154                 | 15.4                                | 60                                   |                                                                   |                |                                       |  |
| X                | 10% of ITP-63A                                 | 8                                 | 103                 | 10.3                                | 60                                   |                                                                   |                |                                       |  |
| Y                | 10% of ITP-63A                                 | 5                                 | 234                 | 23.4                                | 60                                   |                                                                   |                |                                       |  |

| Sweater specimen | Process shrinkage, percent |             |              |               |       | Laundering shrinkage, percent, after 10L and tumble drying |             |              |               |       |
|------------------|----------------------------|-------------|--------------|---------------|-------|------------------------------------------------------------|-------------|--------------|---------------|-------|
|                  | Band                       | Back length | Bottom width | Sleeve length | Chest | Band                                                       | Back length | Bottom width | Sleeve length | Chest |
| W                | 12.7                       | 10.6        | None         | 5.6           | None  | None                                                       | 2.4         | +0.8         | 2.4           | None  |
| X                | 10.7                       | 9.9         | do           | 5.6           | None  | None                                                       | 2.4         | None         | 2.4           | Do.   |
| Y                | 5.7                        | 4.3         | do           | 2.3           | +0.7  | 1.4                                                        | 2.3         | do           | +3.5          | Do.   |
| Untreated        |                            |             |              |               |       | 27.2                                                       | 33.3        | do           |               | 20.4  |

wool blends as well as those on untreated controls are tabulated below. The values show a consistent improvement in fuzziness rating in comparison with the corresponding untreated control specimen, both prior to laundering and after 12 launderings. Wash-and-wear ratings were not adversely affected. Resistance to flex abrasion and flat frosting remain either unchanged or were improved by the treatment.

utes. The procedures of scouring, drying, shearing, and semidecating were similar to those of Example XXII. As to properties, crease retention and wash-and-wear ratings (on pressed specimens) were improved over those of similar fabrics processed in a conventional way. Other values on the treated polyester-wool blends, along with control data, are tabulated below, and show the substantial improvement brought about by the imine-terminated

| Composition of dyed fabric                       | Fuzziness rating |      | Wash-and-wear rating |      | Flat frosting rating (2.5-lb., 1,200 cycles) |     | Resistance to flex abrasion, cycles (1-lb. head, 4-lb. toggle) No L |  |
|--------------------------------------------------|------------------|------|----------------------|------|----------------------------------------------|-----|---------------------------------------------------------------------|--|
|                                                  | No L             | 12 L | 1 L                  | 12 L | No L                                         | Web | Rupture                                                             |  |
| 55% acrylic/45% wool                             | 5                | 4    | 4.5                  | 3.5  | 5                                            | 525 | 800                                                                 |  |
| 55% acrylic/45% wool, untreated control          | 3                | 3    | 4.5                  | 3.5  | 5                                            | 500 | 800                                                                 |  |
| 65% acrylic/30% wool/5% rayon                    | 3-4              | 3    | 4.3                  | 3.0  | 4                                            | 225 | 525                                                                 |  |
| 65% acrylic/30% wool/5% rayon, untreated control | 1                | 1    | 4.5                  | 3.5  | 3                                            | 150 | 300                                                                 |  |
| 70% acrylic/30% wool                             | 4                | 3-4  | 3.5                  | 3.5  | 5                                            | 375 | 575                                                                 |  |
| 70% acrylic/30% wool, untreated control          | 2                | 2    | 3.5                  | 3.5  | 5                                            | 275 | 475                                                                 |  |

### EXAMPLE XXIII

#### Control of fuzz and abrasion of dyed polyester-wool blends by imine-terminated polymer

Each of four 60-yard lengths of colored fabrics of two different polyester-wool blends identified in the accompanying table was padded with a dispersion formulated as follows. An approximately 5.4% dispersion of ITP-63A was made by blending 130 pounds of the thick emulsion (40% ITP-63A) recorded in Example XXII and 100 gallons (approximately 830 pounds) of water. Wet pickup was approximately 50%, the pad pressure being 12 tons. Speed was 25 yards per minute. For the combined step of drying-curing, conditions were 300° F. for 4.5 min-

| Composition of dyed fabrics                                 | Fuzziness rating |      | Resistance to flex abrasion, cycles (1-lb. head, 4-lb. toggle) No L |         |
|-------------------------------------------------------------|------------------|------|---------------------------------------------------------------------|---------|
|                                                             | No L             | 10 L | Web                                                                 | Rupture |
| 55% polyester/45% wool, 6.90 oz./sq. yd.                    | 4-5              | 4-5  | 650                                                                 | 285     |
| 55% polyester/45% wool, 6.90 oz./sq. yd., untreated control | 2                | 3-4  | 525                                                                 | 125     |
| 55% polyester/45% wool, 5.38 oz./sq. yd.                    | 4                | 4-5  | 375                                                                 | 185     |
| 55% polyester/45% wool, 5.38 oz./sq. yd., untreated control | 2                | 3    | 150                                                                 | 100     |
| 70% polyester/30% wool, 6.82 oz./sq. yd.                    | 4                | 5    | 1,050                                                               | 275     |
| 70% polyester/30% wool, 6.82 oz./sq. yd., untreated control | 1-2              | 3    | 650                                                                 | 135     |
| 70% polyester/30% wool, 4.57 oz./sq. yd.                    | 4                | 5    | 500                                                                 | 175     |
| 70% polyester/30% wool, 4.57 oz./sq. yd., untreated control | 3                | 4    | 425                                                                 | 110     |

25 polymer on each polyester-wool blend.

### EXAMPLE XXIV

Control of abrasion and shrinkage of both undyed and dyed fabrics of blends of synthetic fibers with wool by treatment with imine-terminated polymer

Each of eight lengths of fabrics of four kinds of blends of synthetic fibers with wool as identified in the accompanying table was padded with a solution formulated as follows.

35 An approximately 5.5% dispersion of ITP-63A was made by blending 113 pounds of the thick emulsion (40% ITP-63A) recorded in Example XXII and 85 gallons (approximately 705 pounds) of water. Pad pressure was 12 tons, and speed was 15 yards per minute. For the combined step of drying-curing, conditions were 275° F. for 7.5 minutes. The procedures of scouring, drying, shearing, and semidecating for the acrylic-wool blends were similar to those of Example XXII, but the polyester-wool blends were singed before semidecating. "Singeing" means

40 burning off the free projecting fibers from the surface of the cloth, leaving it smooth and bare. Upon evaluation, it was found that crease retention and wash-and-wear ratings (on pressed specimens) were improved over those of similar fabrics processed in a conventional manner. Other data on the treated blends of synthetic fibers and wool, dyed as well as undyed, together with control data, are tabulated below. Definite improvement was effected by the imine-terminated polymer on each wool-containing blend. (Control samples were dyed but otherwise untreated.)

| Composition of fabric  | State   | Yardage treated, percent | Wet pickup, percent | Laundering shrinkage, percent (10-inch markings machine wash, 105° F., tumble dry, low setting) |     |      |     |
|------------------------|---------|--------------------------|---------------------|-------------------------------------------------------------------------------------------------|-----|------|-----|
|                        |         |                          |                     | Resistance to flex abrasion cycles (1 lb X 4-lb.) No L, web                                     |     | 5L   |     |
|                        |         |                          |                     | W                                                                                               | F   | W    | F   |
| 55% polyester/45% wool | Dyed    | 35                       | 52                  | 650                                                                                             | 1.0 | 1.0  | 1.0 |
|                        | Control | Untreated                |                     | 525                                                                                             | 1.5 | 3.0  | 1.5 |
|                        | Undyed  | 35                       | 51                  | 775                                                                                             | 1.5 | 0.5  | 1.5 |
| 70% polyester/30% wool | Dyed    | 35                       | 50                  | 875                                                                                             | 0.5 | 1.0  | 0.5 |
|                        | Control | Untreated                |                     | 775                                                                                             | 0.5 | 2.0  | 0.5 |
|                        | Undyed  | 60                       | 50                  | 1,050                                                                                           | 0.5 | None | 0.5 |
| 55% acrylic/45% wool   | Dyed    | 50                       | 56                  | 650                                                                                             | 1.5 | 1.5  | 2.5 |
|                        | Control | Untreated                |                     | 525                                                                                             | 2.5 | 3.5  | 4.0 |
|                        | Undyed  | 50                       | 55                  | 725                                                                                             | 1.0 | 2.0  | 1.5 |
| 70% acrylic/30% wool   | Dyed    | 50                       | 57                  | 575                                                                                             | 1.5 | 0.5  | 1.5 |
|                        | Control | Untreated                |                     | 425                                                                                             | 2.5 | 2.5  | 2.5 |
|                        | Undyed  | 50                       | 59                  | 500                                                                                             | 1.5 | 1.0  | 1.5 |

**27**  
**EXAMPLE XXV**

Preparation of a polyfunctional compound having (1) a polyester chain as its backbone, and (2) terminal 2-(1-aziridinyl)ethoxy groups



Isocyanate-terminated polyester, wherein  $v=3$  to 4 and  $n=$ about 6

the hydroxyl-terminated polyether into an isocyanate-terminated compound. A 1-liter jar equipped with a stirrer, a thermometer, a dropping funnel, and a vent was charged with 200 grams of polytetramethylene ether glycol dissolved in 200 grams of dichloromethane and cooled to



$-15\pm 5^\circ \text{ C}$ . 4-methyl-m-phenylene diisocyanate (35.4 grams, 0.203 mole) dissolved in 50 grams of dichloro-



Starting materials and the procedure were similar to those of Example XI except as follows: The weight of dichloromethane was 330 grams instead of 100 grams. Instead of ethylenimine, (1-aziridine)ethanol (20.7 grams, 0.238 mole) was added dropwise to the stirred solution at 20 to  $30^\circ \text{ C}$ . The addition was completed within 1 hour. The reaction solution remained homogeneous. One-half hour after termination of the addition, the infrared absorption band was devoid of the isocyanate band (4.3 to 4.5 microns). Analysis revealed an aziridinyl content of 0.15 equivalent per 100 grams of solid (calculated, 0.197 eq./100 g.). The solution was miscible with dimethylformamide.

**EXAMPLE XXVI**

Preparation of a polyfunctional compound having (1) a polytetramethyleneoxy chain as its backbone, and (2) terminal 2-(1-aziridinyl)ethoxy groups

*First stage:*



On the average,  $x=$ about 26 in Example XXVI, and about 13 in Examples XXVII and XXVIII



ICTIT, an isocyanate-terminated intermediate having a backbone derived from a polytetramethyleneoxy chain

*Second stage:*



2-(1-aziridinyl)ethoxy-terminated polytetramethyleneoxy chain

The polytetramethylene ether glycol used as the starting material had an average molecular weight of approximately 1980. The polymer was marketed under the trade name Polymeg by Quaker Oats Co.

The *first stage* of the process consisted of converting

**28**

5 the hydroxyl-terminated polyether into an isocyanate-terminated compound. A 1-liter jar equipped with a stirrer, a thermometer, a dropping funnel, and a vent was charged with 200 grams of polytetramethylene ether glycol dissolved in 200 grams of dichloromethane and cooled to



$-15\pm 5^\circ \text{ C}$ . 4-methyl-m-phenylene diisocyanate (35.4 grams, 0.203 mole) dissolved in 50 grams of dichloro-

25 methane was added. The temperature was allowed to rise to  $25^\circ \text{ C}$ . during 1 hour. The reaction mixture was stored at approximately  $5^\circ \text{ C}$ . for several days.

Next, the *second stage* of adding terminal 2-(1-aziridinyl)ethoxy radicals was carried out. (1-aziridine)ethanol (17.4 grams, 0.20 mole) was added dropwise to 19/20 of the original solution obtained from the first stage. The stirred solution contained 0.19 equivalent of  $-\text{N}=\text{C}=\text{O}$  [determined by a modification of the dibutylamine procedure of W. Sieffken, Liebigs Annalen der Chemie, vol. 562, page 100 (1949)]. The addition was completed in 0.5 hour, during which time the reaction temperature was kept at  $26\pm 2^\circ \text{ C}$ . The solution was stirred for 2 hours longer, after which time the infrared spectrum was devoid of the isocyanate band at 4.3 to 4.5 microns. The solution had an aziridinyl content of 0.076 equivalent per 100 grams of solid (0.084 eq./100 g., calculated). The solution was miscible with dimethylformamide.

**EXAMPLE XXVII**

45 A preparation similar to Example XXVI, but of lower molecular weight

The chemical equations of Example XXVI applied, except that  $x$ , the degree of polymerization, was about 13 on the average. The polytetramethylene ether glycol used in Example XXVII had an average molecular weight of approximately 1020.

In the *first stage*, 200 grams (0.393 equivalent of hydroxyl) of polytetramethylene ether glycol and 68.4 grams (0.393 mole) of 4-methyl-m-phenylene diisocyanate were allowed to interact under conditions similar to those of Example XXVI. Two days later, the isocyanate content

70 was 0.40 equivalent (theoretically 0.393 equivalent).

In the *second stage*, 93% of the isocyanate-terminated intermediate was allowed to react with 34.8 grams (0.4 mole) of (1-aziridine)ethanol in a manner similar to that described in Example XXVI. The aziridinyl content of the product was 0.13 equivalent per 100 grams of solid (0.14 eq./100 g., calculated).

EXAMPLE XXVIII

A preparation similar to Example XXVII, but having terminal 2-(1-aziridinyl)ethylamino groups

For the chemical equation applying to the *first stage*, see Example XXVI,  $x$ =about 13 on the average.

### *Second stage:*



2-(1-aziridinyl)ethylamino - terminated polytetramethyl-  
eneoxy chain

In the first stage, the isocyanate-terminated intermediate (ICTIT) having a backbone derived from a polytetra-



methyleneoxy chain was prepared in a manner similar to that of Example XXVII from polytetramethylene ether.

In the *second stage*, 0.26 equivalent of the isocyanate-terminated intermediate was allowed to react with 11.3 grams (0.26 mole) of ethylenimine in a manner similar to that described in Example XXVI. The aziridinyl content was found to be 0.14 equivalent per 100 grams of solid (theoretically 0.14 eq./100 g.).

### EXAMPLE XXX

A preparation having (1) a complex polyester chain as its backbone, and (2) terminal 1-aziridinyl groups

### *First stage:*



glycol having an average molecular weight of approximately 1020.

In the second stage, 0.31 equivalent of the isocyanate-terminated intermediate which was 79% of the original amount obtained in the first stage was allowed to react with 33.5 grams of 1-(2-aminoethyl)aziridine dissolved in 50 grams of dichloromethane in a manner similar to that described in Example XXVI. The aziridinyl content was found to be 0.17 equivalent per 100 grams of solid. (0.164 eq./100 g. calculated.)

### EXAMPLE XXIX

Preparation of a polyfunctional compound having (1) a residue of ethoxylated glycerol as the central portion of its molecule, and (2) terminal 1-azidinyl groups



wherein  $x+x+z$  is approximately 32.

The ethoxylated glycerol used as starting material had an average molecular weight of 1495. In the *first stage*, 200 grams of the ethoxylated glycerol and 70 grams (0.402 mole) of 4-methyl-m-phenylene diisocyanate were allowed to interact under conditions similar to those of Example XXVI. By analysis at the end of the reaction period, the isocyanate content was found to be 0.42 equivalent (theoretically 0.402 equivalent).

ICTIP, an isocyanate-terminated intermediate having a backbone derived from a complex polyester chain

### 30 Second stage:



As in Example XXV,  $\gamma=3$  to 4, and  $n=$  about 2-8.

40 The first stage of the process was carried out as follows. A mixture of 6.82 grams of ethylene glycol (0.11 mole) and 75 grams of dichloromethane was added quickly to a stirred solution at 0° C. consisting of 200 grams of dichloromethane and 200 grams (0.446 equivalent of isocyanate) of isocyanate-terminated polyester identified in Example XI. Stirring was continued as the reaction mixture was allowed to warm to room temperature. After 2 weeks, the isocyanate content became constant at 0.24 equivalent (calculated, 0.226 equivalent).

For the second stage, a solution of 6.4 grams (0.149 mole) of ethylenimine and 50 grams of dichloromethane was added dropwise within 1 hour at room temperature to 57% of the amount of the product (0.136 equivalent of isocyanate) obtained in the first stage. After a period of 1 day, the infrared spectrum was devoid of the isocyanate band. The reaction solution had an aziridinyl content of 0.11 equivalent per 100 grams of solid (0.12 eq./100 g., calculated; theoretically 0.103 eq. of the desired product per 100 grams of solids). The desired product has a complex polyester backbone terminated at both ends of the molecule by 1-aziridinyl groups.

### EXAMPLE XXXI

## Dimensional stabilization of woolen fabric by treatment with the product of Example XXV

Samples of 100% woolen fabric in a plain weave and weighing 6.15 ounces per square yard were treated according to the quantitative details in the accompanying table with solutions of the product of Example XXVI. A 38% solution of the product in dichloromethane was diluted by dimethylformamide to give the percentages OWB shown in the accompanying table. Solutions were applied by means of a laboratory padder. After padding, the samples were framed at the original dimensions and

dried at approximately 50°C. All samples were cured for 5 minutes. The cured fabric was rinsed in dimethylformamide, then in a 0.1% aqueous solution of p-(1,1,3,3-tetramethylbutyl)phenoxy nona(ethyleneoxy)ethanol again framed to the original dimensions, and dried. Shrinkproofing evaluation was excellent and durable, as is evident from the evaluation results in the accompanying table. The polymer was reactive because of amine-type 1-aziridinyl groups terminating the chain, the center portion of which was a polyester.

### EXAMPLE XXXIII

## Dimensional stabilization of woolen fabric by treatment with the product of Example XXVII

5 The procedure of Example XXXII was repeated using  
 as the reagent the product of Example XXVII, a lower-  
 molecular-weight polymer than had been used in Example  
 XXXII. A 60% solution of the product in dichloro-  
 10 methane was diluted with dimethylformamide to give  
 the percentages OWB shown in the accompanying table.

EXAMPLE XXXII

## Dimensional stabilization of woolen fabric by treatment with the product of Example XXVI

Samples of the woolen fabric identified in Example

Good shrinkproofing resulted with this polymer also having amine-type terminal 1-aziridinyl groups but with a polyalkyleneoxy backbone having a smaller degree of polymerization. The polymer was effective even at low concentration.

XXXI were treated according to the general procedure of that example with the following variations: The reagent was the product of Example XXVI. A 54% solution of it in dichloromethane was diluted with dimethylformamide to give the percentages OWB shown in the accompanying table. After padding, samples (18 by 17 inches) were dried at approximately 65° C. Curing was for 5 minutes, and other quantitative details are in the accompanying table. Excellent shrinkproofing resulted from the use of the reactive polymer having a backbone made up of repeating tetramethyleneoxy units, the molecular chain being terminated by amine-type 1-aziridinyl groups. Even at low concentration, the reagent was very effective.

#### EXAMPLE XXXIV

## Dimensional stabilization of woolen fabric by treatment with the product of Example XXVIII

55 A procedure similar to that of Example XXXII was followed, using as the reagent the product of Example XXVIII, a polymer resembling that used in Example XXXIII except for terminal 2-(1-aziridinyl)ethylamino groups in place of 2-(1-aziridinyl)ethoxy groups. A 45% solution of the product in dichloromethane was diluted 60 with dimethylformamide to give the percentages OWB shown in the accompanying table. Durable shrink-proof-

| Product of Example<br>XXVIII, percent | Cure<br>temp.,<br>°C | Actual<br>weight<br>gain,<br>percent | Warp flex<br>abrasion<br>resistance<br>0.5 x 2 lb.,<br>cycles | Warp<br>stiffi-<br>ness,<br>mg.-cm. | Green<br>filter<br>reflect-<br>ance,<br>percent | Shrinkage, percent |     |     |      |      |
|---------------------------------------|----------------------|--------------------------------------|---------------------------------------------------------------|-------------------------------------|-------------------------------------------------|--------------------|-----|-----|------|------|
|                                       |                      |                                      |                                                               |                                     |                                                 | 5L                 | W   |     |      |      |
| OWB                                   | WPU                  | OWF                                  |                                                               |                                     |                                                 |                    | F   |     |      |      |
| Sample:                               |                      |                                      |                                                               |                                     |                                                 |                    |     |     |      |      |
| B-1-----                              | 3.3                  | 120                                  | 4.0                                                           | 135                                 | 5.4                                             | 1,175              | 510 | 63  | 1.5  | 1.5  |
| B-2-----                              | 3.3                  | 119                                  | 3.9                                                           | 163                                 | 5.3                                             | 915                | 685 | 62  | 1.0  | 1.0  |
| C-1-----                              | 1.7                  | 120                                  | 2.0                                                           | 135                                 | 2.6                                             | 975                | 429 | 387 | 64   | 1.5  |
| C-2-----                              | 1.7                  | 119                                  | 2.0                                                           | 163                                 | 2.9                                             | 725                | 429 | 63  | 1.5  | 1.5  |
| D-1-----                              | 0.9                  | 121                                  | 1.1                                                           | 135                                 | 1.7                                             | 750                | 288 | 64  | 4.0  | 2.5  |
| D-2-----                              | 0.9                  | 118                                  | 1.1                                                           | 163                                 | 1.7                                             | 825                | 307 | 64  | 3.5  | 2.5  |
| Untreated control                     |                      |                                      |                                                               |                                     |                                                 | 815                | 107 | 65  | 22.5 | 11.0 |

ing resulted over a good range of concentrations with this reactive polymer.

It is understood that various other modifications will be apparent to and can readily be made by those skilled

|                   | Product of Example<br>XXVIII, percent |     |     | Cure<br>temp.,<br>°C | Actual<br>weight<br>gain,<br>percent | Warp flex<br>abrasion<br>resistance<br>0.5 x 2 lb.,<br>cycles | Warp<br>stiff-<br>ness,<br>mg.-cm. | Green<br>filter<br>reflect-<br>ance,<br>percent | Shrinkage, percent * |       |
|-------------------|---------------------------------------|-----|-----|----------------------|--------------------------------------|---------------------------------------------------------------|------------------------------------|-------------------------------------------------|----------------------|-------|
|                   | OWB                                   | WPU | OWF |                      |                                      |                                                               |                                    |                                                 | 5L                   |       |
| <b>Sample:</b>    |                                       |     |     |                      |                                      |                                                               |                                    |                                                 |                      |       |
| A-1               | 5.00                                  | 118 | 5.9 | 135                  | 7.0                                  | 1,475                                                         | 2,000                              | 63                                              | 1.5                  | 0.5   |
| A-2               | 5.00                                  | 117 | 5.9 | 163                  | 6.8                                  | 1,250                                                         | 1,700                              | 62                                              | 1.5                  | 0.5   |
| B-1               | 3.33                                  | 114 | 3.8 | 135                  | 3.8                                  | 1,175                                                         | 1,300                              | 63                                              | 1.0                  | 0.5   |
| B-2               | 3.33                                  | 110 | 3.8 | 163                  | 3.5                                  | 1,025                                                         | 1,200                              | 62                                              | 1.5                  | 0.5   |
| C-1               | 1.67                                  | 111 | 1.9 | 135                  | 2.1                                  | 925                                                           | 600                                | 62                                              | 2.5                  | (0.5) |
| C-2               | 1.67                                  | 115 | 1.9 | 163                  | 2.1                                  | 850                                                           | 400                                | 61                                              | 2.5                  | None  |
| D-1               | 0.84                                  | 114 | 1.0 | 135                  | 1.4                                  | 850                                                           | 380                                | 64                                              | 4.5                  | (0.5) |
| D-2               | 0.84                                  | 117 | 1.0 | 163                  | 1.4                                  | 775                                                           | 430                                | 62                                              | 4.5                  | (0.5) |
| Untreated control |                                       |     |     |                      |                                      |                                                               |                                    |                                                 |                      |       |
|                   |                                       |     |     |                      |                                      | 815                                                           | 107                                | 65                                              | 22.5                 | 11.0  |

\* Percentages in parentheses are the opposite of shrinkage.

### EXAMPLE XXXV

## Dimensional stabilization of woolen fabric by treatment with the product of Example XXIX

A procedure similar to that of Example XXXII was followed, using as the product of Example XXIX, a polymer whose central moiety came from ethoxylated glycerol, and having amide-type 1-aziridinyl terminal groups. A 51% solution of the product in dichloromethane was diluted with dimethylformamide to give the percentages OWB shown in the accompanying table. Good results on shrinkproofing are evident.

in the art without departing from the scope and spirit of this invention. Accordingly, it is not intended that the scope of the claims appended hereto be limited to the description set forth herein but rather that the claims be construed as encompassing all the features of patentable novelty which reside in the present invention, including all features which would be treated as equivalents thereof by those skilled in the art to which the invention pertains.

What is claimed is:

**1. A process for improving the dimensional stability of proteinaceous material comprising applying to said pro-**

| Product of Example<br>XXVIII, percent | Cure<br>temp.,<br>°C | Actual<br>weight<br>gain,<br>percent | Warp flex<br>abrasion<br>resistance<br>0.5 x 2 lb.,<br>cycles | Warp<br>stiff-<br>ness,<br>mg.-cm. | Green<br>filter<br>reflect-<br>ance,<br>percent | Shrinkage, percent |     |    |      |      |
|---------------------------------------|----------------------|--------------------------------------|---------------------------------------------------------------|------------------------------------|-------------------------------------------------|--------------------|-----|----|------|------|
|                                       |                      |                                      |                                                               |                                    |                                                 | 5L                 |     |    |      |      |
| OWB                                   | WPU                  | OWF                                  |                                                               |                                    |                                                 | W                  | F   |    |      |      |
| Sample:                               |                      |                                      |                                                               |                                    |                                                 |                    |     |    |      |      |
| A                                     | 5.10                 | 129                                  | 6.6                                                           | 135                                | 7.8                                             | 1,200              | 490 | 62 | 2.0  | 0.5  |
| B                                     | 3.40                 | 124                                  | 4.2                                                           | 135                                | 6.0                                             | 1,000              | 425 | 62 | 2.0  | 0.5  |
| C                                     | 1.70                 | 121                                  | 2.1                                                           | 135                                | 3.5                                             | 975                | 295 | 63 | 4.5  | 0.5  |
| D                                     | 0.85                 | 120                                  | 1.0                                                           | 135                                | 2.5                                             | 1,050              | 260 | 64 | 6.5  | None |
| Untreated control                     |                      |                                      |                                                               |                                    |                                                 | 815                | 107 | 65 | 22.5 | 11.0 |

### EXAMPLE XXXVI

### Dimensional stabilization using the product of Example XXX

A procedure similar to that of Example XXXI was followed, using the product of Example XXX, a polymer whose central moiety was mainly a polyester, and whose terminal groups were amide-type 1-aziridinyl groups. The product was diluted with dimethylformamide to give the percentages OWB shown in the accompanying table. All samples were cured for 5 minutes at approximately 163° C. Upon evaluation, good control of shrinkage was obtained, as is apparent from the accompanying table.

teinaceous material a polyfunctional compound of the formula



wherein

*m* is in integer of from 2 to 3,

A is selected from the group consisting of Az,

—NH—C<sub>a</sub>H<sub>2a</sub>Az, and —O—C<sub>a</sub>H<sub>2a</sub>Az,

*a* is an



TABLE TO EXAMPLE XXXVI

| Product of Example<br>XXX, percent | Shrinkage, percent         |                                                 |                                  |     |      |     |      |      |
|------------------------------------|----------------------------|-------------------------------------------------|----------------------------------|-----|------|-----|------|------|
|                                    | Actual<br>weight<br>gain % | Abrasion resis-<br>tance 0.5 x 2<br>lb., cycles | Warp stiff-<br>ness, mg.-<br>cm. | 1L  | 5L   |     |      |      |
| OWB                                | WPU                        | OWF                                             |                                  | W   | F    | W   | F    |      |
| Wool fabric sample:                |                            |                                                 |                                  |     |      |     |      |      |
| A-----                             | 6.6                        | 5.3                                             | 825                              | 538 | 1.5  | 1.5 | 2.0  | 1.5  |
| B-----                             | 4.4                        | 4.0                                             | 875                              | 258 | 3.5  | 0.5 | 4.0  | None |
| C-----                             | 2.1                        | 3.2                                             | 825                              | 277 | 3.0  | 0.5 | 3.5  | 0.5  |
| Control untreated-----             |                            |                                                 | 900                              | 132 | 10.5 | 3.0 | 21.5 | 12.5 |

wherein

$R^1, R^2, R^3$ , are selected from the group consisting of H and alkyl having from 1 to 4 carbon atoms, J is selected from the group consisting of

- $(-\text{CH}_2-)_x$
- $(-\text{C}_n\text{H}_{2n}\text{O}-)_x\text{C}_n\text{H}_{2n}$
- $(-\text{CH}_2\text{CH}=\text{CHCH}_2-)_u$
- $\left[(-\text{CH}_2-)_n-\text{O}-\text{C}(=\text{O})-\text{CH}_2-\right]_v$
- $[(-\text{CH}_2-)_n-\text{O}-\text{C}(=\text{O})-\text{CH}_2-)_q-\text{C}(=\text{O})-\text{O}]_r(-\text{CH}_2-)_n$
- $-\text{C}_n\text{H}_{2n}(-\text{O C}_n\text{H}_{2n}-)_x\text{O}-\text{L}-\text{O}(-\text{C}_n\text{H}_{2n}\text{O}-)_y\text{C}_n\text{H}_{2n}-$
- $(-\text{C}_n\text{H}_{2n}\text{O}-)_x-\text{CH}_2-\text{HOC}(-\text{O C}_n\text{H}_{2n}-)_y$
- $(-\text{C}_n\text{H}_{2n}\text{O}-)_z-\text{CH}_2$

wherein

a has the meaning given above, x, y and z independently are integers of from about 1 to 100, u is an integer of from about 6 to 100, n is an integer of from 2 to 6, v is an integer of from about 3 to 80, q is an integer of from 3 to 5, r is an integer of from 2 to 35, and L is a divalent alicyclic radical of 3 to 20 carbon atoms,  $\text{C}_2$  to  $\text{C}_{20}$  alkylene, or  $\text{C}_2$  to  $\text{C}_{20}$  alkylene having the chain interrupted by one to ten —O—, —S—, or groups in which

R is H or alkyl having 1 to 5 carbon atoms,

Q is selected from the group consisting of  $-\text{C}_6\text{H}_4-$ ,  $-\text{C}_6\text{H}_3(-\text{CH}_3)-$ ,  $-\text{H}_2\text{CC}_6\text{H}_4\text{CH}_2-$ ,  $\text{C}_6\text{H}_4\text{C}_6\text{H}_4-$ ,  $-\text{C}_6\text{H}_4\text{CH}_2\text{C}_6\text{H}_4-$ ,  $-\text{C}_6\text{H}_3(-\text{CH}_2\text{C}_6\text{H}_5)-$  and  $\text{C}_{10}\text{H}_8-$ ,

said polyfunctional compound being applied from a liquid medium and heating the proteinaceous material having

acids of 2 to 12 carbon atoms and polyalkylenepolyamines of 4 to 20 carbon atoms and 2 to 5 nitrogen atoms.

7. A process as claimed in claim 1 wherein Q is



8. The process of claim 6 wherein about 0.5 to about 2.0 equivalents of co-reactant are present for each aziridinyl group present and the pH of the liquid medium ranges between about 3.0 to about 9.0.

9. The compound of the structure:



A is selected from the group consisting of



m is an integer selected from 2 and 3, Q is methylphenylene,

J is the residue of an aliphatic polyol having from 2 to 4 hydroxyl groups after the removal of from 2 to 4 hydroxyl groups, having a molecular weight ranging between about 14 and 5500.

10. The compound of the structure:



polyfunctional compound applied thereto until the desired dimensional stabilization takes place.

2. A process as claimed in claim 1 wherein said proteinaceous material is wool.

50 wherein v is an integer ranging from 3 to 4, and n is an integer ranging from 2 to 8.

11. The compound of the structure:



3. A process as claimed in claim 1 wherein said polyfunctional material is dissolved in an inert organic solvent.

4. The process of claim 1 wherein the polyfunctional compound is applied from an aqueous emulsion.

5. A process as claimed in claim 1 wherein said proteinaceous material having polyfunctional compound applied thereto is heated at a temperature of about 100 to 200°C.

6. A process as claimed in claim 1 wherein, in addition to said polyfunctional compound there is applied to said proteinaceous material a coreactant selected from the group consisting of saturated aliphatic dicarboxylic

65 wherein x is an integer ranging from 5 to 40.

12. The compound of the structure:



70 wherein x+y+z=approximately 32.

13. The compound of the structure:



wherein  $v$  is an integer ranging from 3 to 4, and  $n$  is an integer ranging from 2 to 8.

14. The compound of the structure:



wherein  $v$  is an integer ranging from 2 to 6, and  $n$  is an integer ranging from 4 to 8. 25

15. The compound of the structure:



wherein  $x$  is an integer ranging from 5 to 40.

16. A process as claimed in claim 6 wherein said poly-

18. A process as claimed in claim 6 wherein the poly-functional compound is of the structures:



functional compound is of the structure:



50 wherein  $n$  is an integer of from 2 to 6;  $q$  is an integer of from 3 to 5; and  $r$  is an integer of from 2 to 35.

19. A process as claimed in claim 6 wherein the poly-functional compound is of the structure:



wherein  $x+y+z=50$ , the co-reactant is a polyalkylene polyamine, and perchloroethylene is present as an inert organic solvent.

17. A process as claimed in claim 6 wherein said poly-functional compound is of the structure:



wherein  $u$  is an integer of from about 6 to 100.

20. A process as claimed in claim 6 wherein the poly-functional compound is of the structure:



wherein  $n$  is an integer of from 2 to 6, and  $v$  is an integer of from 3 to 80.

21. A process as claimed in claim 6 wherein the polyfunctional compound is of the structure:



wherein  $u$  is an integer of from about 6 to 100.

22. A process as claimed in claim 6 wherein the polyfunctional compound is of the structure:



wherein  $v$  is an integer of from about 3 to 80, and  $n$  is an integer of from 2 to 6.

23. A process as claimed in claim 6 wherein the polyfunctional compound is of the structure:



wherein  $x$  is an integer of from about 1 to 100.

24. A process as claimed in claim 6 wherein the polyfunctional compound is of the structure:



wherein  $x$  is an integer of from about 1 to 100.

25. A process as claimed in claim 6 wherein the polyfunctional compound is of the structure:



wherein  $x+y+z$  = approximately 32.

26. A process as claimed in claim 1 wherein the polyfunctional compound is of the structure:



3,523,750

41

wherein  $v$  is an integer of from 3 to 4, and  $n$  is an integer of from 2 to 8.

References Cited

UNITED STATES PATENTS

3,225,013 12/1965 Fram ----- 260—78  
3,165,375 1/1965 Tesord ----- 8—127.6

42

3,223,681 12/1965 Rambosek ----- 260—77.5  
3,115,474 12/1963 Smith ----- 260—2

DONALD LEVY, Primary Examiner

B. BETTIS, Assistant Examiner

U.S. Cl. X.R.

5 8—128; 117—141; 260—2, 77.5, 239, 240

UNITED STATES PATENT OFFICE  
CERTIFICATE OF CORRECTION

Patent No. 3,523,750 Dated August 11, 1970

Inventor(s) Giuliana C. Tesoro

It is certified that error appears in the above-identified patent and that said Letters Patent are hereby corrected as shown below:

Col. 3, line 13, "be" should be -- by --; Col. 10, line 3, delete "as that used in connection with the aziridine com" and substitute -- from which it is deposited on the woolen textile --; Col. 12, formula at line 12, end of formula,



Col. 14, in the chart beginning at line 6, the last number in last column should be clarified to read -- 4,150 --; Col. 21, Table of Example XVII, Sample H under Wet Pickup Percent "138" should read -- 128 --; Col. 23, Table of Example XIX, Sample D-2 under Wet Pickup Percent, "13.0" should read -- 130 --; Col. 24, Table of Example XX, Sample C under Shrinkage Percent 5L - F, " 3.5" should read -- 2.5 --; Col. 24, Table of Example XX, Sample D under same heading "0.5" should read -- +0.5 --; Col. 27, second formula below the first  ring



line 43, " micable" should read -- miscible --; Col. 29, at the beginning of First Stage of Formula of Example XXX,

UNITED STATES PATENT OFFICE  
CERTIFICATE OF CORRECTION

Patent No. 3,523,750 Dated August 11, 1970

Inventor(s) Giuliana C. Tesoro --2--

It is certified that error appears in the above-identified patent and that said Letters Patent are hereby corrected as shown below:

Page 2 - Continued

" HOCH<sub>2</sub>OH<sub>2</sub>OH " should read -- HOCH<sub>2</sub>CH<sub>2</sub>OH -- ; Col. 29,  
at the bottom of the first  ring (Second Stage Formula) of  
Example XXX

"  " should read --  -- ; Col. 31, in the  
CH<sub>2</sub>

Table of Example XXXII at bottom of page, "Product of Example  
XXVIII Percent" should read -- Product of Example XXVI Percent--;  
Col. 31 Table of Example XXXIII at center of page "Product of  
Example XXVIII Percent" should read -- Product of Example XXVII  
Percent -- ; Col. 33, second Table on page (of Example XXXV),  
"Product of Example XXVIII" should read -- Product of Example  
XXIX -- ; Col. 33, the Table at bottom of page (Example  
XXXVI) "Abrasion Resistance 0.5' x 2 lb. cycles" should read  
-- Warp Flex Abrasion Resistance 0.5 x 2 lb. cycles --; Claim 1,  
Col. 35, line 31, after "or" add -- -N- -- ; Claim 15,  
R

Col. 37, before the second  ring of the formula

" -CN-- " should read -- -CN-- --;

Claim 18, Col. 38 at the end of the formula

UNITED STATES PATENT OFFICE  
CERTIFICATE OF CORRECTION

Patent No. 3,523,750

Dated August 11, 1970

--3--

Inventor(s) Giuliana C. Tesoro

It is certified that error appears in the above-identified patent and that said Letters Patent are hereby corrected as shown below:

Page 3 - Continued

" NHCON  " should read -- NHCON  --; Claim 19,

Col. 38, at the beginning of the formula "  " should read --  --; Claim 19, Col. 38 before the first 

ring " H<sub>2</sub>C- " should read -- H<sub>3</sub>C- --; Claim 20,

Col. 39, at the end of the formula "  " should read --  --; Claim 22, Col. 39, after the first 

ring in the formula "  " should read --  --

Signed and sealed this 9th day of July 1974.

(SEAL)  
Attest:

McCOY M. GIBSON, JR.  
Attesting Officer

C. MARSHALL DANN  
Commissioner of Patents